



US009682425B2

(12) **United States Patent**  
**Xu et al.**

(10) **Patent No.:** **US 9,682,425 B2**  
(45) **Date of Patent:** **\*Jun. 20, 2017**

(54) **COATED METALLIC POWDER AND  
METHOD OF MAKING THE SAME**

(75) Inventors: **Zhiyue Xu**, Cypress, TX (US); **Gaurav Agrawal**, Aurora, CO (US); **Bobby Salinas**, Sugar Land, TX (US)

(73) Assignee: **BAKER HUGHES INCORPORATED**, Houston, TX (US)

(\*) Notice: Subject to any disclaimer, the term of this patent is extended or adjusted under 35 U.S.C. 154(b) by 669 days.

This patent is subject to a terminal disclaimer.

(21) Appl. No.: **12/633,686**

(22) Filed: **Dec. 8, 2009**

(65) **Prior Publication Data**

US 2011/0135953 A1 Jun. 9, 2011

(51) **Int. Cl.**  
**B22F 1/02** (2006.01)

(52) **U.S. Cl.**  
CPC ..... **B22F 1/025** (2013.01); **B22F 1/02** (2013.01); **B22F 2998/10** (2013.01); **B22F 2999/00** (2013.01); **Y10T 428/12028** (2015.01); **Y10T 428/2991** (2015.01)

(58) **Field of Classification Search**

None

See application file for complete search history.

(56)

**References Cited**

U.S. PATENT DOCUMENTS

|             |         |              |
|-------------|---------|--------------|
| 1,468,905 A | 9/1923  | Herman       |
| 2,189,697 A | 2/1940  | Baker        |
| 2,222,233 A | 11/1940 | Mize         |
| 2,225,143 A | 12/1940 | Baker et al. |
| 2,238,895 A | 4/1941  | Gage         |

(Continued)

FOREIGN PATENT DOCUMENTS

|    |           |         |
|----|-----------|---------|
| CN | 1076968   | 10/1993 |
| CN | 1079234 A | 12/1993 |

(Continued)

OTHER PUBLICATIONS

Abdoulaye Seyni, Nadine Le Bolay, Sonia Molina-Boisseau, "On the interest of using degradable fillers in co-ground composite materials", Powder Technology 190, (2009) pp. 176-184.

(Continued)

*Primary Examiner* — Adam Krupicka

(74) *Attorney, Agent, or Firm* — Cantor Colburn, LLP

(57) **ABSTRACT**

A metallic powder is disclosed. The metallic powder includes a plurality of metallic powder particles. Each powder particle includes a particle core. The particle core includes a core material comprising Mg, Al, Zn or Mn, or a combination thereof, having a melting temperature ( $T_p$ ). Each powder particle also includes a metallic coating layer disposed on the particle core. The metallic coating layer includes a metallic coating material having a melting temperature ( $T_c$ ). The powder particles are configured for solid-state sintering to one another at a predetermined sintering temperature ( $T_s$ ), and  $T_s$  is less than  $T_p$  and  $T_c$ .

**17 Claims, 13 Drawing Sheets**



(56)

## References Cited

## U.S. PATENT DOCUMENTS

|               |         |                       |             |         |                       |
|---------------|---------|-----------------------|-------------|---------|-----------------------|
| 2,261,292 A   | 11/1941 | Salnikov              | 4,690,796 A | 9/1987  | Paliwal               |
| 2,294,648 A   | 9/1942  | Ansel et al.          | 4,693,863 A | 9/1987  | Del Corso et al.      |
| 2,301,624 A   | 11/1942 | Holt                  | 4,703,807 A | 11/1987 | Weston                |
| 2,352,993 A   | 7/1944  | Albertson             | 4,706,753 A | 11/1987 | Ohkochi et al.        |
| 2,394,843 A   | 2/1946  | Cooke et al.          | 4,708,202 A | 11/1987 | Sukup et al.          |
| 2,672,199 A   | 3/1948  | McKenna               | 4,708,208 A | 11/1987 | Halbardier            |
| 2,753,941 A   | 7/1956  | Hebard et al.         | 4,709,761 A | 12/1987 | Setterberg, Jr.       |
| 2,754,910 A   | 7/1956  | Derrick et al.        | 4,714,116 A | 12/1987 | Brunner               |
| 2,933,136 A   | 4/1960  | Ayers et al.          | 4,716,964 A | 1/1988  | Erbstoesser et al.    |
| 2,983,634 A   | 5/1961  | Budininkas et al.     | 4,719,971 A | 1/1988  | Owens                 |
| 3,057,405 A   | 10/1962 | Mallinger             | 4,721,159 A | 1/1988  | Ohkochi et al.        |
| 3,066,391 A   | 12/1962 | Vordahl               | 4,724,599 A | 4/1988  | Shilling              |
| 3,106,959 A   | 10/1963 | Huitt et al.          | 4,738,599 A | 5/1988  | Condit et al.         |
| 3,142,338 A   | 7/1964  | Brown                 | 4,741,973 A | 9/1988  | Kupsa                 |
| 3,152,009 A   | 10/1964 | DeLong                | 4,768,588 A | 10/1988 | Jaeckel               |
| 3,196,949 A   | 7/1965  | Thomas                | 4,775,598 A | 11/1988 | Wyatt                 |
| 3,242,988 A   | 3/1966  | McGuire et al.        | 4,784,226 A | 2/1989  | Halbardier            |
| 3,316,748 A   | 5/1967  | Lang et al.           | 4,805,699 A | 4/1989  | Jenkins               |
| 3,326,291 A   | 6/1967  | Zandmer et al.        | 4,817,725 A | 5/1989  | Streich et al.        |
| 3,343,537 A   | 9/1967  | Solis                 | 4,834,184 A | 6/1989  | Johnson et al.        |
| 3,347,317 A   | 10/1967 | Solis                 | 4,863 H     | 6/1989  | Brandell et al.       |
| 3,347,714 A   | 10/1967 | Broverman et al.      | 4,880,059 A | 11/1989 | Porter et al.         |
| 3,390,724 A   | 7/1968  | Caldwell              | 4,889,187 A | 12/1989 | Terrell et al.        |
| 3,395,758 A   | 8/1968  | Kelly et al.          | 4,890,675 A | 1/1990  | Dew                   |
| 3,406,101 A   | 10/1968 | Kilpatrick            | 4,901,794 A | 2/1990  | Baugh et al.          |
| 3,416,918 A   | 12/1968 | Henry                 | 4,909,320 A | 3/1990  | Hebert et al.         |
| 3,465,181 A   | 9/1969  | Colby et al.          | 4,929,415 A | 5/1990  | Okazaki               |
| 3,489,218 A   | 1/1970  | Means                 | 4,932,474 A | 6/1990  | Schroeder, Jr. et al. |
| 3,513,230 A * | 5/1970  | Hammar et al. ....    | 4,938,309 A | 7/1990  | Emdy                  |
| 3,602,305 A   | 8/1971  | Kisling               | 4,938,809 A | 7/1990  | Das et al.            |
| 3,637,446 A   | 1/1972  | Elliott et al.        | 4,944,351 A | 7/1990  | Eriksen et al.        |
| 3,645,331 A   | 2/1972  | Maurer et al.         | 4,949,788 A | 8/1990  | Szarka et al.         |
| 3,660,049 A   | 5/1972  | Benjamin              | 4,952,902 A | 12/1990 | Okazaki et al.        |
| 3,765,484 A   | 10/1973 | Hamby, Jr. et al.     | 4,975,412 A | 12/1990 | Miller                |
| 3,768,563 A   | 10/1973 | Blount                | 4,977,958 A | 1/1991  | Carmody et al.        |
| 3,775,823 A   | 12/1973 | Adolph et al.         | 4,981,177 A | 1/1991  | Mueller et al.        |
| 3,816,080 A   | 6/1974  | Bomford et al.        | 4,986,361 A | 1/1991  | Regazzoni et al.      |
| 3,878,889 A   | 4/1975  | Seabourn              | 4,997,622 A | 3/1991  | Walker, Sr. et al.    |
| 3,894,850 A   | 7/1975  | Kovalchuk et al.      | 5,006,044 A | 4/1991  | Springer              |
| 3,924,677 A   | 12/1975 | Prenner et al.        | 5,010,955 A | 4/1991  | Pittard et al.        |
| 4,010,583 A   | 3/1977  | Highborg              | 5,036,921 A | 8/1991  | Cochran               |
| 4,039,717 A   | 8/1977  | Titus                 | 5,048,611 A | 9/1991  | Tselesin              |
| 4,050,529 A   | 9/1977  | Tagirov et al.        | 5,049,165 A | 10/1991 | DeLucchia             |
| 4,157,732 A   | 6/1979  | Fonner                | 5,061,323 A | 11/1991 | Walker, Sr. et al.    |
| 4,248,307 A   | 2/1981  | Silberman et al.      | 5,063,775 A | 12/1991 | Faure et al.          |
| 4,284,137 A   | 8/1981  | Taylor                | 5,073,207 A | 12/1991 | Brisco et al.         |
| 4,292,377 A   | 9/1981  | Petersen et al.       | 5,074,361 A | 12/1991 | Bourell et al.        |
| 4,372,384 A   | 2/1983  | Kinney                | 5,076,869 A | 1/1992  | Okazaki               |
| 4,373,584 A   | 2/1983  | Silberman et al.      | 5,084,088 A | 2/1992  | Chang et al.          |
| 4,373,952 A   | 2/1983  | Parent                | 5,087,304 A | 2/1992  | Pittard et al.        |
| 4,374,543 A   | 2/1983  | Richardson            | 5,090,480 A | 3/1992  | Bode                  |
| 4,384,616 A   | 5/1983  | Dellinger             | 5,095,988 A | 4/1992  | Heijnen               |
| 4,395,440 A   | 7/1983  | Abe et al.            | 5,103,911 A | 6/1992  | Mueller et al.        |
| 4,399,871 A   | 8/1983  | Adkins et al.         | 5,117,915 A | 11/1992 | Wu et al.             |
| 4,407,368 A   | 10/1983 | Erbstoesser           | 5,161,614 A | 12/1992 | Sanjurjo et al.       |
| 4,422,508 A   | 12/1983 | Rutledge, Jr. et al.  | 5,171,734 A | 1/1993  | Giroux et al.         |
| 4,452,311 A   | 6/1984  | Speegle et al.        | 5,178,216 A | 1/1993  | Mueller et al.        |
| 4,475,729 A   | 10/1984 | Costigan              | 5,181,571 A | 1/1993  | Walker, Sr. et al.    |
| 4,498,543 A   | 2/1985  | Pye et al.            | 5,183,631 A | 2/1993  | Kugimiya et al.       |
| 4,499,048 A   | 2/1985  | Hanejko               | 5,188,182 A | 2/1993  | Echols, III et al.    |
| 4,499,049 A   | 2/1985  | Hanejko               | 5,188,183 A | 2/1993  | Hopmann et al.        |
| 4,524,825 A   | 6/1985  | Fore                  | 5,204,055 A | 4/1993  | Sachs et al.          |
| 4,526,840 A   | 7/1985  | Jerabek               | 5,222,867 A | 6/1993  | Walker, Sr. et al.    |
| 4,534,414 A   | 8/1985  | Pringle               | 5,226,483 A | 7/1993  | Williamson, Jr.       |
| 4,539,175 A   | 9/1985  | Lichti et al.         | 5,228,518 A | 7/1993  | Wilson et al.         |
| 4,554,986 A   | 11/1985 | Jones                 | 5,234,055 A | 8/1993  | Cornette              |
| 4,619,699 A   | 10/1986 | Petkovic-Luton et al. | 5,252,365 A | 10/1993 | White                 |
| 4,640,354 A   | 2/1987  | Boisson               | 5,253,714 A | 10/1993 | Davis et al.          |
| 4,664,962 A   | 5/1987  | DesMarais, Jr.        | 5,271,468 A | 12/1993 | Streich et al.        |
| 4,668,470 A   | 5/1987  | Gilman et al.         | 5,282,509 A | 2/1994  | Schurr, III           |
| 4,673,549 A   | 6/1987  | Ecer                  | 5,292,478 A | 3/1994  | Scorey                |
| 4,674,572 A   | 6/1987  | Gallus                | 5,293,940 A | 3/1994  | Hromas et al.         |
| 4,678,037 A   | 7/1987  | Smith                 | 5,304,260 A | 4/1994  | Aikawa et al.         |
| 4,681,133 A   | 7/1987  | Weston                | 5,304,588 A | 4/1994  | Boysen et al.         |
| 4,688,641 A   | 8/1987  | Knieriem              | 5,309,874 A | 5/1994  | Willermet et al.      |
|               |         |                       | 5,310,000 A | 5/1994  | Arterbury et al.      |

| (56)                  | References Cited |                         |              |         |                    |  |
|-----------------------|------------------|-------------------------|--------------|---------|--------------------|--|
| U.S. PATENT DOCUMENTS |                  |                         |              |         |                    |  |
| 5,316,598 A           | 5/1994           | Chang et al.            | 6,050,340 A  | 4/2000  | Scott              |  |
| 5,318,746 A           | 6/1994           | Lashmore                | 6,069,313 A  | 5/2000  | Kay                |  |
| 5,352,522 A           | 10/1994          | Kugimiya et al.         | 6,076,600 A  | 6/2000  | Vick, Jr. et al.   |  |
| 5,380,473 A           | 1/1995           | Bogue et al.            | 6,079,496 A  | 6/2000  | Hirth              |  |
| 5,387,380 A           | 2/1995           | Cima et al.             | 6,085,837 A  | 7/2000  | Massinon et al.    |  |
| 5,392,860 A           | 2/1995           | Ross                    | 6,095,247 A  | 8/2000  | Streich et al.     |  |
| 5,394,236 A           | 2/1995           | Murnick                 | 6,119,783 A  | 9/2000  | Parker et al.      |  |
| 5,394,941 A           | 3/1995           | Venditto et al.         | 6,142,237 A  | 11/2000 | Christmas et al.   |  |
| 5,398,754 A           | 3/1995           | Dinhoble                | 6,161,622 A  | 12/2000 | Robb et al.        |  |
| 5,407,011 A           | 4/1995           | Layout                  | 6,167,970 B1 | 1/2001  | Stout et al.       |  |
| 5,409,555 A           | 4/1995           | Fujita et al.           | 6,170,583 B1 | 1/2001  | Boyce              |  |
| 5,411,082 A           | 5/1995           | Kennedy                 | 6,173,779 B1 | 1/2001  | Smith              |  |
| 5,417,285 A           | 5/1995           | Van Buskirk et al.      | 6,176,323 B1 | 1/2001  | Weirich et al.     |  |
| 5,425,424 A           | 6/1995           | Reinhardt et al.        | 6,189,616 B1 | 2/2001  | Gano et al.        |  |
| 5,427,177 A           | 6/1995           | Jordan, Jr. et al.      | 6,189,618 B1 | 2/2001  | Beeman et al.      |  |
| 5,435,392 A           | 7/1995           | Kennedy                 | 6,213,202 B1 | 4/2001  | Read, Jr.          |  |
| 5,439,051 A           | 8/1995           | Kennedy et al.          | 6,220,350 B1 | 4/2001  | Brothers et al.    |  |
| 5,454,430 A           | 10/1995          | Kennedy et al.          | 6,220,357 B1 | 4/2001  | Carmichael         |  |
| 5,456,317 A           | 10/1995          | Hood, III et al.        | 6,228,904 B1 | 5/2001  | Yadav et al.       |  |
| 5,456,327 A           | 10/1995          | Denton et al.           | 6,237,688 B1 | 5/2001  | Burleson et al.    |  |
| 5,464,062 A           | 11/1995          | Blizzard, Jr.           | 6,238,280 B1 | 5/2001  | Ritt et al.        |  |
| 5,472,048 A           | 12/1995          | Kennedy et al.          | 6,241,021 B1 | 6/2001  | Bowling            |  |
| 5,474,131 A           | 12/1995          | Jordan, Jr. et al.      | 6,248,399 B1 | 6/2001  | Hehmann            |  |
| 5,477,923 A           | 12/1995          | Jordan, Jr. et al.      | 6,250,392 B1 | 6/2001  | Muth               |  |
| 5,479,986 A           | 1/1996           | Gano et al.             | 6,261,432 B1 | 7/2001  | Huber et al.       |  |
| 5,506,055 A           | 4/1996           | Dorfman et al.          | 6,273,187 B1 | 8/2001  | Voisin, Jr. et al. |  |
| 5,507,439 A           | 4/1996           | Story                   | 6,276,452 B1 | 8/2001  | Davis et al.       |  |
| 5,511,620 A           | 4/1996           | Baugh et al.            | 6,276,457 B1 | 8/2001  | Moffatt et al.     |  |
| 5,524,699 A           | 6/1996           | Cook                    | 6,279,656 B1 | 8/2001  | Sinclair et al.    |  |
| 5,526,880 A           | 6/1996           | Jordan, Jr. et al.      | 6,287,445 B1 | 9/2001  | Lashmore et al.    |  |
| 5,526,881 A           | 6/1996           | Martin et al.           | 6,302,205 B1 | 10/2001 | Ryll               |  |
| 5,529,746 A           | 6/1996           | Knoss et al.            | 6,315,041 B1 | 11/2001 | Carlisle et al.    |  |
| 5,533,573 A           | 7/1996           | Jordan, Jr. et al.      | 6,315,050 B2 | 11/2001 | Vaynshteyn et al.  |  |
| 5,536,485 A           | 7/1996           | Kume et al.             | 6,325,148 B1 | 12/2001 | Trahan et al.      |  |
| 5,558,153 A           | 9/1996           | Holcombe et al.         | 6,328,110 B1 | 12/2001 | Joubert            |  |
| 5,601,924 A           | 2/1997           | Beane                   | 6,341,653 B1 | 1/2002  | Firmaniuk et al.   |  |
| 5,607,017 A           | 3/1997           | Owens et al.            | 6,341,747 B1 | 1/2002  | Schmidt et al.     |  |
| 5,623,993 A           | 4/1997           | Van Buskirk et al.      | 6,349,766 B1 | 2/2002  | Bussear et al.     |  |
| 5,623,994 A           | 4/1997           | Robinson                | 6,354,372 B1 | 3/2002  | Carisella et al.   |  |
| 5,636,691 A           | 6/1997           | Hendrickson et al.      | 6,354,379 B2 | 3/2002  | Miszewski et al.   |  |
| 5,641,023 A           | 6/1997           | Ross et al.             | 6,357,322 B1 | 3/2002  | Dolan et al.       |  |
| 5,647,444 A           | 7/1997           | Williams                | 6,371,206 B1 | 4/2002  | Mills              |  |
| 5,665,289 A           | 9/1997           | Chung et al.            | 6,372,346 B1 | 4/2002  | Toth               |  |
| 5,677,372 A           | 10/1997          | Yamamoto et al.         | 6,382,244 B2 | 5/2002  | Vann               |  |
| 5,685,372 A           | 11/1997          | Gano                    | 6,390,195 B1 | 5/2002  | Nguyen et al.      |  |
| 5,701,576 A           | 12/1997          | Fujita et al.           | 6,390,200 B1 | 5/2002  | Allamon et al.     |  |
| 5,707,214 A           | 1/1998           | Schmidt                 | 6,394,180 B1 | 5/2002  | Berscheidt et al.  |  |
| 5,709,269 A           | 1/1998           | Head                    | 6,394,185 B1 | 5/2002  | Constien           |  |
| 5,720,344 A           | 2/1998           | Newman                  | 6,397,950 B1 | 6/2002  | Streich et al.     |  |
| 5,728,195 A           | 3/1998           | Eastman et al.          | 6,401,547 B1 | 6/2002  | Hatfield et al.    |  |
| 5,765,639 A           | 6/1998           | Muth                    | 6,403,210 B1 | 6/2002  | Stuivinga et al.   |  |
| 5,772,735 A           | 6/1998           | Sehgal et al.           | 6,408,946 B1 | 6/2002  | Marshall et al.    |  |
| 5,782,305 A           | 7/1998           | Hicks                   | 6,419,023 B1 | 7/2002  | George et al.      |  |
| 5,797,454 A           | 8/1998           | Hipp                    | 6,439,313 B1 | 8/2002  | Thomeer et al.     |  |
| 5,826,652 A           | 10/1998          | Tapp                    | 6,446,717 B1 | 9/2002  | White et al.       |  |
| 5,826,661 A           | 10/1998          | Parker et al.           | 6,457,525 B1 | 10/2002 | Scott              |  |
| 5,829,520 A           | 11/1998          | Johnson                 | 6,467,546 B2 | 10/2002 | Allamon et al.     |  |
| 5,836,396 A           | 11/1998          | Norman                  | 6,470,965 B1 | 10/2002 | Winzer             |  |
| 5,857,521 A           | 1/1999           | Ross et al.             | 6,491,097 B1 | 12/2002 | ONeal et al.       |  |
| 5,881,816 A           | 3/1999           | Wright                  | 6,491,116 B2 | 12/2002 | Berscheidt et al.  |  |
| 5,896,819 A           | 4/1999           | Turila et al.           | 6,513,598 B2 | 2/2003  | Moore et al.       |  |
| 5,902,424 A           | 5/1999           | Fujita et al.           | 6,513,600 B2 | 2/2003  | Ross               |  |
| 5,934,372 A           | 8/1999           | Muth                    | 6,535,604 B1 | 3/2003  | Provencal et al.   |  |
| 5,941,309 A           | 8/1999           | Appleton                | 6,540,033 B1 | 4/2003  | Sullivan et al.    |  |
| 5,960,881 A           | 10/1999          | Allamon et al.          | 6,543,543 B2 | 4/2003  | Muth               |  |
| 5,985,466 A           | 11/1999          | Atarashi et al.         | 6,561,275 B2 | 5/2003  | Glass et al.       |  |
| 5,988,287 A           | 11/1999          | Jordan, Jr. et al.      | 6,588,507 B2 | 7/2003  | Dusterhoft et al.  |  |
| 5,990,051 A           | 11/1999          | Ischy et al.            | 6,591,915 B2 | 7/2003  | Burris et al.      |  |
| 5,992,452 A           | 11/1999          | Nelson, II              | 6,601,648 B2 | 8/2003  | Ebinger            |  |
| 5,992,520 A           | 11/1999          | Schultz et al.          | 6,601,650 B2 | 8/2003  | Sundararajan       |  |
| 6,007,314 A           | 12/1999          | Nelson, II              | 6,609,569 B2 | 8/2003  | Howlett et al.     |  |
| 6,024,915 A *         | 2/2000           | Kume et al. .... 419/48 | 6,612,826 B1 | 9/2003  | Bauer et al.       |  |
| 6,032,735 A           | 3/2000           | Echols                  | 6,613,383 B1 | 9/2003  | George et al.      |  |
| 6,036,777 A           | 3/2000           | Sachs                   | 6,619,400 B2 | 9/2003  | Brunet             |  |
| 6,047,773 A           | 4/2000           | Zeltmann et al.         | 6,630,008 B1 | 10/2003 | Meeks, III et al.  |  |
|                       |                  |                         | 6,634,428 B2 | 10/2003 | Krauss et al.      |  |
|                       |                  |                         | 6,662,886 B2 | 12/2003 | Russell            |  |
|                       |                  |                         | 6,675,889 B1 | 1/2004  | Mullins et al.     |  |
|                       |                  |                         | 6,699,305 B2 | 3/2004  | Myrick             |  |

| (56)                  | References Cited |                      |              |         |                          |
|-----------------------|------------------|----------------------|--------------|---------|--------------------------|
| U.S. PATENT DOCUMENTS |                  |                      |              |         |                          |
| 6,712,153 B2          | 3/2004           | Turley et al.        | 7,320,365 B2 | 1/2008  | Pia                      |
| 6,712,797 B1          | 3/2004           | Southern, Jr.        | 7,322,412 B2 | 1/2008  | Badalamenti et al.       |
| 6,713,177 B2          | 3/2004           | George et al.        | 7,322,417 B2 | 1/2008  | Rytlewski et al.         |
| 6,715,541 B2          | 4/2004           | Pedersen et al.      | 7,325,617 B2 | 2/2008  | Murray                   |
| 6,719,051 B2          | 4/2004           | Hailey, Jr. et al.   | 7,328,750 B2 | 2/2008  | Swor et al.              |
| 6,755,249 B2          | 6/2004           | Robison et al.       | 7,331,388 B2 | 2/2008  | Vilela et al.            |
| 6,769,491 B2          | 8/2004           | Zimmerman et al.     | 7,337,854 B2 | 3/2008  | Horn et al.              |
| 6,776,228 B2          | 8/2004           | Pedersen et al.      | 7,346,456 B2 | 3/2008  | Le Bemadjiel             |
| 6,779,599 B2          | 8/2004           | Mullins et al.       | 7,350,582 B2 | 4/2008  | McKeachnie et al.        |
| 6,799,638 B2          | 10/2004          | Butterfield, Jr.     | 7,353,879 B2 | 4/2008  | Todd et al.              |
| 6,810,960 B2          | 11/2004          | Pia                  | 7,360,593 B2 | 4/2008  | Constien                 |
| 6,817,414 B2          | 11/2004          | Lee                  | 7,360,597 B2 | 4/2008  | Blaisdell                |
| 6,831,044 B2          | 12/2004          | Constien             | 7,363,970 B2 | 4/2008  | Corre et al.             |
| 6,883,611 B2          | 4/2005           | Smith et al.         | 7,373,978 B2 | 5/2008  | Barry et al.             |
| 6,887,297 B2          | 5/2005           | Winter et al.        | 7,380,600 B2 | 6/2008  | Willberg et al.          |
| 6,896,049 B2          | 5/2005           | Moyes                | 7,387,158 B2 | 6/2008  | Murray et al.            |
| 6,896,061 B2          | 5/2005           | Hriscu et al.        | 7,387,165 B2 | 6/2008  | Lopez de Cardenas et al. |
| 6,899,176 B2          | 5/2005           | Hailey, Jr. et al.   | 7,392,841 B2 | 7/2008  | Murray et al.            |
| 6,899,777 B2          | 5/2005           | Vaidyanathan et al.  | 7,401,648 B2 | 7/2008  | Richard                  |
| 6,908,516 B2          | 6/2005           | Hehmann et al.       | 7,416,029 B2 | 8/2008  | Telfer et al.            |
| 6,913,827 B2          | 7/2005           | George et al.        | 7,422,058 B2 | 9/2008  | O'Malley                 |
| 6,926,086 B2          | 8/2005           | Patterson et al.     | 7,426,964 B2 | 9/2008  | Lynde et al.             |
| 6,932,159 B2          | 8/2005           | Hovem                | 7,441,596 B2 | 10/2008 | Wood et al.              |
| 6,939,388 B2          | 9/2005           | Angeliu              | 7,445,049 B2 | 11/2008 | Howard et al.            |
| 6,945,331 B2          | 9/2005           | Patel                | 7,451,815 B2 | 11/2008 | Hailey, Jr.              |
| 6,951,331 B2          | 10/2005          | Haughom et al.       | 7,451,817 B2 | 11/2008 | Reddy et al.             |
| 6,959,759 B2          | 11/2005          | Doane et al.         | 7,461,699 B2 | 12/2008 | Richard et al.           |
| 6,973,970 B2          | 12/2005          | Johnston et al.      | 7,464,764 B2 | 12/2008 | Xu                       |
| 6,973,973 B2          | 12/2005          | Howard et al.        | 7,472,750 B2 | 1/2009  | Walker et al.            |
| 6,983,796 B2          | 1/2006           | Bayne et al.         | 7,478,676 B2 | 1/2009  | East, Jr. et al.         |
| 6,986,390 B2          | 1/2006           | Doane et al.         | 7,503,390 B2 | 3/2009  | Gomez                    |
| 7,013,989 B2          | 3/2006           | Hammond et al.       | 7,503,399 B2 | 3/2009  | Badalamenti et al.       |
| 7,013,998 B2          | 3/2006           | Ray et al.           | 7,509,993 B1 | 3/2009  | Turng et al.             |
| 7,017,664 B2          | 3/2006           | Walker et al.        | 7,510,018 B2 | 3/2009  | Williamson et al.        |
| 7,017,677 B2          | 3/2006           | Keshavan et al.      | 7,513,311 B2 | 4/2009  | Gramstad et al.          |
| 7,021,389 B2          | 4/2006           | Bishop et al.        | 7,516,791 B2 | 4/2009  | Bryant et al.            |
| 7,025,146 B2          | 4/2006           | King et al.          | 7,527,103 B2 | 5/2009  | Huang et al.             |
| 7,028,778 B2          | 4/2006           | Krywitsky            | 7,537,825 B1 | 5/2009  | Wardle et al.            |
| 7,044,230 B2          | 5/2006           | Starr et al.         | 7,552,777 B2 | 6/2009  | Murray et al.            |
| 7,048,812 B2          | 5/2006           | Bettles et al.       | 7,552,779 B2 | 6/2009  | Murray                   |
| 7,049,272 B2          | 5/2006           | Sinclair et al.      | 7,559,357 B2 | 7/2009  | Clem                     |
| 7,051,805 B2          | 5/2006           | Doane et al.         | 7,575,062 B2 | 8/2009  | East, Jr.                |
| 7,059,410 B2          | 6/2006           | Bousche et al.       | 7,579,087 B2 | 8/2009  | Maloney et al.           |
| 7,090,027 B1          | 8/2006           | Williams             | 7,591,318 B2 | 9/2009  | Tilghman                 |
| 7,093,664 B2          | 8/2006           | Todd et al.          | 7,600,572 B2 | 10/2009 | Slup et al.              |
| 7,096,945 B2          | 8/2006           | Richards et al.      | 7,604,049 B2 | 10/2009 | Vaidya et al.            |
| 7,096,946 B2          | 8/2006           | Jasser et al.        | 7,604,055 B2 | 10/2009 | Richard et al.           |
| 7,097,807 B1          | 8/2006           | Meeks, III et al.    | 7,607,476 B2 | 10/2009 | Tom et al.               |
| 7,097,906 B2          | 8/2006           | Gardner              | 7,617,871 B2 | 11/2009 | Surjaatmadja et al.      |
| 7,108,080 B2          | 9/2006           | Tessari et al.       | 7,635,023 B2 | 12/2009 | Goldberg et al.          |
| 7,111,682 B2          | 9/2006           | Blaisdell            | 7,640,988 B2 | 1/2010  | Phi et al.               |
| 7,128,145 B2          | 10/2006          | Mickey               | 7,661,480 B2 | 2/2010  | Al-Anazi                 |
| 7,141,207 B2          | 11/2006          | Jandeska, Jr. et al. | 7,661,481 B2 | 2/2010  | Todd et al.              |
| 7,150,326 B2          | 12/2006          | Bishop et al.        | 7,703,510 B2 | 4/2010  | Xu                       |
| 7,163,066 B2          | 1/2007           | Lehr                 | 7,703,511 B2 | 4/2010  | Buyers et al.            |
| 7,165,622 B2          | 1/2007           | Hirth et al.         | 7,708,078 B2 | 5/2010  | Stoesz                   |
| 7,168,494 B2          | 1/2007           | Starr et al.         | 7,709,421 B2 | 5/2010  | Jones et al.             |
| 7,174,963 B2          | 2/2007           | Bertelsen            | 7,712,541 B2 | 5/2010  | Loretz et al.            |
| 7,182,135 B2          | 2/2007           | Szarka               | 7,723,272 B2 | 5/2010  | Crews et al.             |
| 7,188,559 B1          | 3/2007           | Vecchio              | 7,726,406 B2 | 6/2010  | Xu                       |
| 7,210,527 B2          | 5/2007           | Walker et al.        | 7,735,578 B2 | 6/2010  | Loehr et al.             |
| 7,210,533 B2          | 5/2007           | Starr et al.         | 7,743,836 B2 | 6/2010  | Cook et al.              |
| 7,217,311 B2          | 5/2007           | Hong et al.          | 7,752,971 B2 | 7/2010  | Loehr                    |
| 7,234,530 B2          | 6/2007           | Gass                 | 7,757,773 B2 | 7/2010  | Rytlewski                |
| 7,250,188 B2          | 7/2007           | Dodelet et al.       | 7,762,342 B2 | 7/2010  | Richard et al.           |
| 7,252,162 B2          | 8/2007           | Akinlade et al.      | 7,770,652 B2 | 8/2010  | Barnett                  |
| 7,255,172 B2          | 8/2007           | Johnson              | 7,771,289 B2 | 8/2010  | Palumbo et al.           |
| 7,255,178 B2          | 8/2007           | Slup et al.          | 7,775,284 B2 | 8/2010  | Richards et al.          |
| 7,264,060 B2          | 9/2007           | Wills                | 7,775,285 B2 | 8/2010  | Surjaatmadja et al.      |
| 7,267,172 B2          | 9/2007           | Hofman               | 7,775,286 B2 | 8/2010  | Duphorne                 |
| 7,267,178 B2          | 9/2007           | Krywitsky            | 7,784,543 B2 | 8/2010  | Johnson                  |
| 7,270,186 B2          | 9/2007           | Johnson              | 7,793,714 B2 | 9/2010  | Johnson                  |
| 7,287,592 B2          | 10/2007          | Surjaatmadja et al.  | 7,793,820 B2 | 9/2010  | Hirano et al.            |
| 7,311,152 B2          | 12/2007          | Howard et al.        | 7,798,225 B2 | 9/2010  | Giroux et al.            |
| 7,316,274 B2          | 1/2008           | Xu et al.            | 7,798,226 B2 | 9/2010  | Themig                   |

| (56)                  | References Cited |                     |                   |         |                      |        |  |
|-----------------------|------------------|---------------------|-------------------|---------|----------------------|--------|--|
| U.S. PATENT DOCUMENTS |                  |                     |                   |         |                      |        |  |
| 7,798,236 B2          | 9/2010           | McKeachnie et al.   | 2002/0000319 A1   | 1/2002  | Brunet               |        |  |
| 7,806,189 B2          | 10/2010          | Frazier             | 2002/0007948 A1   | 1/2002  | Bayne et al.         |        |  |
| 7,806,192 B2          | 10/2010          | Foster et al.       | 2002/0014268 A1   | 2/2002  | Vann                 |        |  |
| 7,810,553 B2          | 10/2010          | Cruickshank et al.  | 2002/0020527 A1   | 2/2002  | Kilaas et al.        |        |  |
| 7,810,567 B2          | 10/2010          | Daniels et al.      | 2002/0047058 A1   | 4/2002  | Verhoff et al.       |        |  |
| 7,819,198 B2          | 10/2010          | Birckhead et al.    | 2002/0066572 A1   | 6/2002  | Muth                 |        |  |
| 7,828,055 B2          | 11/2010          | Willauer et al.     | 2002/0092654 A1   | 7/2002  | Coronado et al.      |        |  |
| 7,833,944 B2          | 11/2010          | Munoz et al.        | 2002/0096365 A1   | 7/2002  | Berscheidt et al.    |        |  |
| 7,849,927 B2          | 12/2010          | Herrera             | 2002/0104616 A1   | 8/2002  | De et al.            |        |  |
| 7,851,016 B2          | 12/2010          | Arbab et al.        | 2002/0108756 A1   | 8/2002  | Harrall et al.       |        |  |
| 7,855,168 B2          | 12/2010          | Fuller et al.       | 2002/0136904 A1   | 9/2002  | Glass et al.         |        |  |
| 7,861,779 B2          | 1/2011           | Vestavik            | 2002/0139541 A1   | 10/2002 | Sheffield et al.     |        |  |
| 7,861,781 B2          | 1/2011           | D'Arcy              | 2002/0162661 A1   | 11/2002 | Krauss et al.        |        |  |
| 7,874,365 B2          | 1/2011           | East, Jr. et al.    | 2003/0019639 A1   | 1/2003  | MacKay               |        |  |
| 7,878,253 B2          | 2/2011           | Stowe et al.        | 2003/0037925 A1   | 2/2003  | Walker et al.        |        |  |
| 7,896,091 B2          | 3/2011           | Williamson et al.   | 2003/0060374 A1   | 3/2003  | Cooke, Jr.           |        |  |
| 7,897,063 B1          | 3/2011           | Perry et al.        | 2003/0075326 A1   | 4/2003  | Ebinger              |        |  |
| 7,900,696 B1          | 3/2011           | Nish et al.         | 2003/0104147 A1   | 6/2003  | Bretschneider et al. |        |  |
| 7,900,703 B2          | 3/2011           | Clark et al.        | 2003/0111728 A1   | 6/2003  | Thai et al.          |        |  |
| 7,909,096 B2          | 3/2011           | Clark et al.        | 2003/0127013 A1   | 7/2003  | Zavitsanos et al.    |        |  |
| 7,909,104 B2          | 3/2011           | Bjorgum             | 2003/0141060 A1   | 7/2003  | Hailey et al.        |        |  |
| 7,909,110 B2          | 3/2011           | Sharma et al.       | 2003/0141061 A1   | 7/2003  | Hailey et al.        |        |  |
| 7,909,115 B2          | 3/2011           | Grove et al.        | 2003/0141079 A1   | 7/2003  | Doane et al.         |        |  |
| 7,913,765 B2          | 3/2011           | Crow et al.         | 2003/0150614 A1   | 8/2003  | Brown et al.         |        |  |
| 7,931,093 B2          | 4/2011           | Foster et al.       | 2003/0155114 A1   | 8/2003  | Pedersen et al.      |        |  |
| 7,938,191 B2          | 5/2011           | Vaidya              | 2003/0155115 A1   | 8/2003  | Pedersen et al.      |        |  |
| 7,946,335 B2          | 5/2011           | Bewlay et al.       | 2003/0159828 A1   | 8/2003  | Howard et al.        |        |  |
| 7,946,340 B2          | 5/2011           | Surjaatmadja et al. | 2003/0164237 A1   | 9/2003  | Butterfield          |        |  |
| 7,958,940 B2          | 6/2011           | Jameson             | 2003/0183391 A1   | 10/2003 | Hriscu et al.        |        |  |
| 7,963,331 B2          | 6/2011           | Surjaatmadja et al. | 2003/0226668 A1   | 12/2003 | Zimmerman et al.     |        |  |
| 7,963,340 B2          | 6/2011           | Gramstad et al.     | 2004/0005483 A1   | 1/2004  | Lin                  |        |  |
| 7,963,342 B2          | 6/2011           | George              | 2004/0020832 A1   | 2/2004  | Richards et al.      |        |  |
| 7,980,300 B2          | 7/2011           | Roberts et al.      | 2004/0031605 A1   | 2/2004  | Mickey               |        |  |
| 7,987,906 B1          | 8/2011           | Troy                | 2004/0045723 A1   | 3/2004  | Slup et al.          |        |  |
| 7,992,763 B2          | 8/2011           | Vecchio et al.      | 2004/0055758 A1   | 3/2004  | Brezinski et al.     |        |  |
| 8,020,619 B1          | 9/2011           | Robertson et al.    | 2004/0058167 A1   | 3/2004  | Arbab et al.         |        |  |
| 8,020,620 B2          | 9/2011           | Daniels et al.      | 2004/0069502 A1   | 4/2004  | Luke                 |        |  |
| 8,025,104 B2          | 9/2011           | Cooke, Jr.          | 2004/0089449 A1   | 5/2004  | Walton et al.        |        |  |
| 8,028,767 B2          | 10/2011          | Radford et al.      | 2004/0094297 A1   | 5/2004  | Malone et al.        |        |  |
| 8,033,331 B2          | 10/2011          | Themig              | 2004/0154806 A1   | 8/2004  | Bode et al.          |        |  |
| 8,039,422 B1          | 10/2011          | Al-Zahraei          | 2004/0159428 A1   | 8/2004  | Hammond et al.       |        |  |
| 8,056,628 B2          | 11/2011          | Whitsitt et al.     | 2004/0159446 A1   | 8/2004  | Haugen et al.        |        |  |
| 8,056,638 B2          | 11/2011          | Clayton et al.      | 2004/0182583 A1   | 9/2004  | Doane et al.         |        |  |
| 8,109,340 B2          | 2/2012           | Doane et al.        | 2004/0216868 A1   | 11/2004 | Owen, Sr.            |        |  |
| 8,127,856 B1          | 3/2012           | Nish                | 2004/0231845 A1   | 11/2004 | Cooke, Jr.           |        |  |
| 8,153,052 B2          | 4/2012           | Jackson et al.      | 2004/0251025 A1   | 12/2004 | Giroux et al.        |        |  |
| 8,163,060 B2          | 4/2012           | Imanishi et al.     | 2004/0256109 A1   | 12/2004 | Johnson              |        |  |
| 8,211,247 B2          | 7/2012           | Marya et al.        | 2004/0256157 A1   | 12/2004 | Tessari et al.       |        |  |
| 8,211,248 B2          | 7/2012           | Marya               | 2004/0261993 A1   | 12/2004 | Nguyen               |        |  |
| 8,226,740 B2          | 7/2012           | Chaumonnot et al.   | 2004/0261994 A1   | 12/2004 | Nguyen et al.        |        |  |
| 8,230,731 B2          | 7/2012           | Dyer et al.         | 2005/0034876 A1   | 2/2005  | Doane et al.         |        |  |
| 8,231,947 B2          | 7/2012           | Vaidya et al.       | 2005/0051329 A1   | 3/2005  | Blaisdell            |        |  |
| 8,263,178 B2          | 9/2012           | Boulos et al.       | 2005/0064247 A1   | 3/2005  | Sane et al.          |        |  |
| 8,276,670 B2          | 10/2012          | Patel               | 2005/0069449 A1   | 3/2005  | Jackson et al.       |        |  |
| 8,277,974 B2          | 10/2012          | Kumar et al.        | 2005/0074612 A1   | 4/2005  | Eklund et al.        |        |  |
| 8,327,931 B2          | 12/2012          | Agrawal et al.      | 2005/0098313 A1   | 5/2005  | Atkins et al.        |        |  |
| 8,403,037 B2          | 3/2013           | Agrawal et al.      | 2005/0102255 A1   | 5/2005  | Bultman              |        |  |
| 8,413,727 B2          | 4/2013           | Holmes              | 2005/0106316 A1   | 5/2005  | Rigney et al.        |        |  |
| 8,425,651 B2          | 4/2013           | Xu et al.           | 2005/0126334 A1   | 6/2005  | Mirchandani          |        |  |
| 8,459,347 B2          | 6/2013           | Stout               | 2005/0161212 A1   | 7/2005  | Leismer et al.       |        |  |
| 8,490,689 B1          | 7/2013           | McClinton et al.    | 2005/0161224 A1   | 7/2005  | Starr et al.         |        |  |
| 8,535,604 B1 *        | 9/2013           | Baker .....         | 2005/0165149 A1   | 7/2005  | Chanak et al.        |        |  |
|                       |                  | B22F 1/0003         | 2005/0194143 A1   | 9/2005  | Xu et al.            |        |  |
|                       |                  | 419/10              | 2005/0199401 A1   | 9/2005  | Patel et al.         |        |  |
|                       |                  |                     | 2005/0205264 A1   | 9/2005  | Starr et al.         |        |  |
|                       |                  |                     | 2005/0205265 A1   | 9/2005  | Todd et al.          |        |  |
|                       |                  |                     | 2005/0205266 A1   | 9/2005  | Todd et al.          |        |  |
|                       |                  |                     | 2005/0235757 A1   | 10/2005 | De Jonge et al.      |        |  |
| 8,573,295 B2          | 11/2013          | Johnson             | 2005/0241824 A1   | 11/2005 | Burris, II et al.    |        |  |
| 8,631,876 B2          | 1/2014           | Xu et al.           | 2005/0241825 A1   | 11/2005 | Burris, II et al.    |        |  |
| 8,956,660 B2          | 2/2015           | Launag et al.       | 2005/0257936 A1   | 11/2005 | Lehr                 |        |  |
| 9,079,246 B2          | 7/2015           | Xu et al.           | 2005/0268746 A1   | 12/2005 | Abkowitz et al.      |        |  |
| 9,080,098 B2          | 7/2015           | Xu et al.           | 2005/0269097 A1   | 12/2005 | Towler               |        |  |
| 9,090,955 B2          | 7/2015           | Xu et al.           | 2005/0275143 A1   | 12/2005 | Toth                 |        |  |
| 9,101,978 B2          | 8/2015           | Xu et al.           | 2005/0279501 A1   | 12/2005 | Surjaatmadja et al.  |        |  |
| 9,243,475 B2          | 1/2016           | Xu                  | 2006/0012087 A1   | 1/2006  | Matsuda et al.       |        |  |
| 9,260,935 B2          | 2/2016           | Murphree et al.     | 2006/0013350 A1   | 1/2006  | Akers                |        |  |
| 2001/0040180 A1       | 11/2001          | Wittebrood et al.   | 2006/0045787 A1 * | 3/2006  | Jandeska et al. .... | 419/47 |  |
| 2001/0045285 A1       | 11/2001          | Russell             | 2006/0057479 A1   | 3/2006  | Niimi et al.         |        |  |
| 2001/0045288 A1       | 11/2001          | Allamon et al.      |                   |         |                      |        |  |

| (56)                  | References Cited  |                          |                             |
|-----------------------|-------------------|--------------------------|-----------------------------|
| U.S. PATENT DOCUMENTS |                   |                          |                             |
| 2006/0081378 A1       | 4/2006            | Howard et al.            |                             |
| 2006/0102871 A1       | 5/2006            | Wang et al.              |                             |
| 2006/0108114 A1       | 5/2006            | Johnson et al.           |                             |
| 2006/0108126 A1       | 5/2006            | Horn et al.              |                             |
| 2006/0110615 A1       | 5/2006            | Karim et al.             |                             |
| 2006/0116696 A1       | 6/2006            | Odermatt et al.          |                             |
| 2006/0124310 A1       | 6/2006            | Lopez de Cardenas et al. |                             |
| 2006/0124312 A1       | 6/2006            | Rytlewski et al.         |                             |
| 2006/0131011 A1       | 6/2006            | Lynde et al.             |                             |
| 2006/0131031 A1       | 6/2006            | McKeachnie et al.        |                             |
| 2006/0131081 A1       | 6/2006            | Mirchandani et al.       |                             |
| 2006/0144515 A1       | 7/2006            | Tada et al.              |                             |
| 2006/0150770 A1       | 7/2006            | Freim et al.             |                             |
| 2006/0151178 A1       | 7/2006            | Howard et al.            |                             |
| 2006/0153728 A1       | 7/2006            | Schoenung et al.         |                             |
| 2006/0162927 A1       | 7/2006            | Walker et al.            |                             |
| 2006/0169453 A1       | 8/2006            | Savery et al.            |                             |
| 2006/0186602 A1       | 8/2006            | Martin et al.            |                             |
| 2006/0207763 A1       | 9/2006            | Hofman et al.            |                             |
| 2006/0213670 A1       | 9/2006            | Bishop et al.            |                             |
| 2006/0231253 A1       | 10/2006           | Vilela et al.            |                             |
| 2006/0283592 A1       | 12/2006           | Sierra et al.            |                             |
| 2007/0017674 A1       | 1/2007            | Blaisdell                |                             |
| 2007/0017675 A1       | 1/2007            | Hammami et al.           |                             |
| 2007/0029082 A1       | 2/2007            | Giroux et al.            |                             |
| 2007/0039161 A1       | 2/2007            | Garcia                   |                             |
| 2007/0039741 A1       | 2/2007            | Hailey                   |                             |
| 2007/0044958 A1       | 3/2007            | Rytlewski et al.         |                             |
| 2007/0044966 A1       | 3/2007            | Davies et al.            |                             |
| 2007/0051521 A1       | 3/2007            | Fike et al.              |                             |
| 2007/0053785 A1       | 3/2007            | Hetz et al.              |                             |
| 2007/0054101 A1       | 3/2007            | Sigalas et al.           |                             |
| 2007/0057415 A1       | 3/2007            | Katagiri et al.          |                             |
| 2007/0062644 A1       | 3/2007            | Nakamura et al.          |                             |
| 2007/0074873 A1       | 4/2007            | McKeachnie et al.        |                             |
| 2007/0102199 A1       | 5/2007            | Smith et al.             |                             |
| 2007/0107899 A1       | 5/2007            | Werner et al.            |                             |
| 2007/0107908 A1       | 5/2007            | Vaidya et al.            |                             |
| 2007/0108060 A1       | 5/2007            | Park                     |                             |
| 2007/0119600 A1       | 5/2007            | Slup et al.              |                             |
| 2007/0131912 A1       | 6/2007            | Simone et al.            |                             |
| 2007/0134496 A1       | 6/2007            | Ka                       |                             |
| 2007/0151009 A1       | 7/2007            | Conrad et al.            |                             |
| 2007/0151769 A1       | 7/2007            | Slutz et al.             |                             |
| 2007/0169935 A1       | 7/2007            | Akbar et al.             |                             |
| 2007/0181224 A1       | 8/2007            | Marya et al.             |                             |
| 2007/0185655 A1       | 8/2007            | Le Bemadjiel             |                             |
| 2007/0187095 A1       | 8/2007            | Walker et al.            |                             |
| 2007/0207182 A1       | 9/2007            | Weber et al.             |                             |
| 2007/0221373 A1       | 9/2007            | Murray                   |                             |
| 2007/0221384 A1       | 9/2007            | Murray                   |                             |
| 2007/0227745 A1       | 10/2007           | Roberts et al.           |                             |
| 2007/0259994 A1       | 11/2007           | Tour et al.              |                             |
| 2007/0261862 A1       | 11/2007           | Murray                   |                             |
| 2007/0272411 A1       | 11/2007           | Lopez De Cardenas et al. |                             |
| 2007/0272413 A1       | 11/2007           | Rytlewski et al.         |                             |
| 2007/0277979 A1       | 12/2007           | Todd et al.              |                             |
| 2007/0284109 A1       | 12/2007           | East et al.              |                             |
| 2007/0284112 A1       | 12/2007           | Magne et al.             |                             |
| 2007/0299510 A1       | 12/2007           | Venkatarman et al.       |                             |
| 2008/0011473 A1       | 1/2008            | Wood et al.              |                             |
| 2008/0020923 A1       | 1/2008            | Debe et al.              |                             |
| 2008/0047707 A1       | 2/2008            | Boney et al.             |                             |
| 2008/0060810 A9       | 3/2008            | Nguyen et al.            |                             |
| 2008/0066923 A1       | 3/2008            | Xu                       |                             |
| 2008/0066924 A1       | 3/2008            | Xu                       |                             |
| 2008/0078553 A1       | 4/2008            | George                   |                             |
| 2008/0081866 A1       | 4/2008            | Gong et al.              |                             |
| 2008/0093073 A1       | 4/2008            | Bustos et al.            |                             |
| 2008/0099209 A1       | 5/2008            | Loretz et al.            |                             |
| 2008/0105438 A1       | 5/2008            | Jordan et al.            |                             |
| 2008/0115932 A1       | 5/2008            | Cooke                    |                             |
| 2008/0121390 A1       | 5/2008            | O'Malley et al.          |                             |
| 2008/0121436 A1       | 5/2008            | Slay et al.              |                             |
| 2008/0127475 A1       | 6/2008            | Griffo                   |                             |
|                       | 2008/0135249 A1   | 6/2008                   | Fripp et al.                |
|                       | 2008/0149325 A1   | 6/2008                   | Crawford                    |
|                       | 2008/0149345 A1   | 6/2008                   | Marya et al.                |
|                       | 2008/0149351 A1   | 6/2008                   | Marya et al.                |
|                       | 2008/0169105 A1   | 7/2008                   | Williamson et al.           |
|                       | 2008/0169130 A1   | 7/2008                   | Norman et al.               |
|                       | 2008/0179060 A1   | 7/2008                   | Surjaatmadja et al.         |
|                       | 2008/0179104 A1   | 7/2008                   | Zhang et al.                |
|                       | 2008/0196801 A1   | 8/2008                   | Zhao et al.                 |
|                       | 2008/0202764 A1   | 8/2008                   | Clayton et al.              |
|                       | 2008/0202814 A1   | 8/2008                   | Lyons et al.                |
|                       | 2008/0210473 A1   | 9/2008                   | Zhang et al.                |
|                       | 2008/0216383 A1   | 9/2008                   | Pierick et al.              |
|                       | 2008/0223586 A1   | 9/2008                   | Barnett                     |
|                       | 2008/0223587 A1   | 9/2008                   | Cherewyk                    |
|                       | 2008/0236829 A1   | 10/2008                  | Lynde                       |
|                       | 2008/0236842 A1   | 10/2008                  | Bhavsar et al.              |
|                       | 2008/0248205 A1   | 10/2008                  | Blanchet et al.             |
|                       | 2008/0248413 A1   | 10/2008                  | Ishii et al.                |
|                       | 2008/0264205 A1   | 10/2008                  | Zeng et al.                 |
|                       | 2008/0264594 A1   | 10/2008                  | Lohmueller et al.           |
|                       | 2008/0277109 A1   | 11/2008                  | Vaidya                      |
|                       | 2008/0277980 A1 * | 11/2008                  | Koda et al. .... 297/215.16 |
|                       | 2008/0282924 A1   | 11/2008                  | Saenger et al.              |
|                       | 2008/0296024 A1   | 12/2008                  | Huang et al.                |
|                       | 2008/0302538 A1   | 12/2008                  | Hofman                      |
|                       | 2008/0314581 A1   | 12/2008                  | Brown                       |
|                       | 2008/0314588 A1   | 12/2008                  | Langlais et al.             |
|                       | 2009/0038858 A1   | 2/2009                   | Griffo et al.               |
|                       | 2009/0044946 A1   | 2/2009                   | Schasteen et al.            |
|                       | 2009/0044949 A1   | 2/2009                   | King et al.                 |
|                       | 2009/0050334 A1   | 2/2009                   | Marya et al.                |
|                       | 2009/0056934 A1   | 3/2009                   | Xu                          |
|                       | 2009/0065216 A1   | 3/2009                   | Frazier                     |
|                       | 2009/0074603 A1   | 3/2009                   | Chan et al.                 |
|                       | 2009/0084553 A1   | 4/2009                   | Rytlewski et al.            |
|                       | 2009/0084556 A1   | 4/2009                   | Richards et al.             |
|                       | 2009/0084600 A1   | 4/2009                   | Severance                   |
|                       | 2009/0090440 A1   | 4/2009                   | Kellett                     |
|                       | 2009/0107684 A1   | 4/2009                   | Cooke                       |
|                       | 2009/0114381 A1   | 5/2009                   | Stroobants                  |
|                       | 2009/0114382 A1   | 5/2009                   | Grove et al.                |
|                       | 2009/0126436 A1   | 5/2009                   | Fly et al.                  |
|                       | 2009/0139720 A1   | 6/2009                   | Frazier                     |
|                       | 2009/0145666 A1   | 6/2009                   | Radford et al.              |
|                       | 2009/0151949 A1   | 6/2009                   | Marya et al.                |
|                       | 2009/0152009 A1   | 6/2009                   | Slay et al.                 |
|                       | 2009/0155616 A1   | 6/2009                   | Thamida et al.              |
|                       | 2009/0159289 A1   | 6/2009                   | Avant et al.                |
|                       | 2009/0178808 A1   | 7/2009                   | Williamson et al.           |
|                       | 2009/0194273 A1   | 8/2009                   | Surjaatmadja et al.         |
|                       | 2009/0205841 A1   | 8/2009                   | Kluge et al.                |
|                       | 2009/0211770 A1   | 8/2009                   | Nutley et al.               |
|                       | 2009/0226340 A1   | 9/2009                   | Marya                       |
|                       | 2009/0226704 A1   | 9/2009                   | Kauppinen et al.            |
|                       | 2009/0242202 A1   | 10/2009                  | Rispler et al.              |
|                       | 2009/0242208 A1   | 10/2009                  | Bolding                     |
|                       | 2009/0242214 A1   | 10/2009                  | Foster et al.               |
|                       | 2009/0255667 A1   | 10/2009                  | Clem et al.                 |
|                       | 2009/0255684 A1   | 10/2009                  | Bolding                     |
|                       | 2009/0255686 A1   | 10/2009                  | Richard et al.              |
|                       | 2009/0260817 A1   | 10/2009                  | Gambier et al.              |
|                       | 2009/0266548 A1   | 10/2009                  | Olsen et al.                |
|                       | 2009/0272544 A1   | 11/2009                  | Giroux et al.               |
|                       | 2009/0283270 A1   | 11/2009                  | Langeslag                   |
|                       | 2009/0293672 A1   | 12/2009                  | Mirchandani et al.          |
|                       | 2009/0301730 A1   | 12/2009                  | Gweily                      |
|                       | 2009/0305131 A1   | 12/2009                  | Kumar et al.                |
|                       | 2009/0308588 A1   | 12/2009                  | Howell et al.               |
|                       | 2009/0317556 A1   | 12/2009                  | Macary                      |
|                       | 2009/0317622 A1   | 12/2009                  | Huang et al.                |
|                       | 2010/0003536 A1   | 1/2010                   | Smith et al.                |
|                       | 2010/0012385 A1   | 1/2010                   | Drivdahl et al.             |
|                       | 2010/0015002 A1   | 1/2010                   | Barrera et al.              |
|                       | 2010/0015469 A1   | 1/2010                   | Romanowski et al.           |
|                       | 2010/0025255 A1   | 2/2010                   | Su et al.                   |
|                       | 2010/0032151 A1   | 2/2010                   | Duphorne                    |
|                       | 2010/0034857 A1   | 2/2010                   | Launag et al.               |
|                       | 2010/0038076 A1   | 2/2010                   | Spray et al.                |

(56)

## References Cited

## U.S. PATENT DOCUMENTS

|                 |         |                          |                 |         |                  |
|-----------------|---------|--------------------------|-----------------|---------|------------------|
| 2010/0038595 A1 | 2/2010  | Imholt et al.            | 2012/0145389 A1 | 6/2012  | Fitzpatrick, Jr. |
| 2010/0040180 A1 | 2/2010  | Kim et al.               | 2012/0168152 A1 | 7/2012  | Casciaro         |
| 2010/0044041 A1 | 2/2010  | Smith et al.             | 2012/0177905 A1 | 7/2012  | Seals et al.     |
| 2010/0051278 A1 | 3/2010  | Mytopher et al.          | 2012/0205120 A1 | 8/2012  | Howell           |
| 2010/0055491 A1 | 3/2010  | Vecchio et al.           | 2012/0205872 A1 | 8/2012  | Reinhardt et al. |
| 2010/0055492 A1 | 3/2010  | Barsoum et al.           | 2012/0211239 A1 | 8/2012  | Kritzler et al.  |
| 2010/0089583 A1 | 4/2010  | Xu et al.                | 2012/0234546 A1 | 9/2012  | Xu et al.        |
| 2010/0089587 A1 | 4/2010  | Stout                    | 2012/0234547 A1 | 9/2012  | O'Malley et al.  |
| 2010/0101803 A1 | 4/2010  | Clayton et al.           | 2012/0267101 A1 | 10/2012 | Cooke, Jr.       |
| 2010/0116495 A1 | 5/2010  | Spray                    | 2012/0292053 A1 | 11/2012 | Xu et al.        |
| 2010/0122817 A1 | 5/2010  | Surjaatmadja et al.      | 2012/0318513 A1 | 12/2012 | Mazyar et al.    |
| 2010/0139930 A1 | 6/2010  | Patel et al.             | 2013/0004847 A1 | 1/2013  | Kumar et al.     |
| 2010/0200230 A1 | 8/2010  | East, Jr. et al.         | 2013/0008671 A1 | 1/2013  | Booth et al.     |
| 2010/0236793 A1 | 9/2010  | Bjorgum                  | 2013/0025409 A1 | 1/2013  | Xu               |
| 2010/0236794 A1 | 9/2010  | Duan et al.              | 2013/0029886 A1 | 1/2013  | Mazyar et al.    |
| 2010/0243254 A1 | 9/2010  | Murphy et al.            | 2013/0032357 A1 | 2/2013  | Mazyar et al.    |
| 2010/0252273 A1 | 10/2010 | Duphorine                | 2013/0048304 A1 | 2/2013  | Agrawal et al.   |
| 2010/0252280 A1 | 10/2010 | Swor et al.              | 2013/0048305 A1 | 2/2013  | Xu et al.        |
| 2010/0270031 A1 | 10/2010 | Patel                    | 2013/0052472 A1 | 2/2013  | Xu               |
| 2010/0276136 A1 | 11/2010 | Evans et al.             | 2013/0081814 A1 | 4/2013  | Gaudette et al.  |
| 2010/0276159 A1 | 11/2010 | Mailand et al.           | 2013/0084643 A1 | 4/2013  | Commarieu et al. |
| 2010/0282338 A1 | 11/2010 | Gerrard et al.           | 2013/0105159 A1 | 5/2013  | Alvarez et al.   |
| 2010/0282469 A1 | 11/2010 | Richard et al.           | 2013/0126190 A1 | 5/2013  | Mazyar et al.    |
| 2010/0294510 A1 | 11/2010 | Holmes                   | 2013/0133897 A1 | 5/2013  | Baihly et al.    |
| 2010/0297432 A1 | 11/2010 | Sherman et al.           | 2013/0146144 A1 | 6/2013  | Joseph et al.    |
| 2010/0304182 A1 | 12/2010 | Facchini et al.          | 2013/0146302 A1 | 6/2013  | Gaudette et al.  |
| 2010/0314105 A1 | 12/2010 | Rose                     | 2013/0168257 A1 | 7/2013  | Mazyar et al.    |
| 2010/0314126 A1 | 12/2010 | Kellner                  | 2013/0186626 A1 | 7/2013  | Aitken et al.    |
| 2010/0319427 A1 | 12/2010 | Lohbeck                  | 2013/0240200 A1 | 9/2013  | Frazier          |
| 2010/0319870 A1 | 12/2010 | Bewlay et al.            | 2013/0240203 A1 | 9/2013  | Frazier          |
| 2010/0326650 A1 | 12/2010 | Tran et al.              | 2013/0299185 A1 | 11/2013 | Xu et al.        |
| 2011/0005773 A1 | 1/2011  | Dusterhoff et al.        | 2013/0299192 A1 | 11/2013 | Xu et al.        |
| 2011/0036592 A1 | 2/2011  | Fay                      | 2013/0300066 A1 | 11/2013 | Xu et al.        |
| 2011/0048743 A1 | 3/2011  | Stafford et al.          | 2013/0319668 A1 | 12/2013 | Tschetter et al. |
| 2011/0052805 A1 | 3/2011  | Bordere et al.           | 2013/0327540 A1 | 12/2013 | Hamid et al.     |
| 2011/0056692 A1 | 3/2011  | Lopez de Cardenas et al. | 2014/0014339 A1 | 1/2014  | O'Malley et al.  |
| 2011/0056702 A1 | 3/2011  | Sharma et al.            | 2014/0027128 A1 | 1/2014  | Johnson          |
| 2011/0067872 A1 | 3/2011  | Agrawal                  | 2014/0060834 A1 | 3/2014  | Quintero et al.  |
| 2011/0067889 A1 | 3/2011  | Marya et al.             | 2014/0116711 A1 | 5/2014  | Tang et al.      |
| 2011/0067890 A1 | 3/2011  | Themig                   | 2014/0262327 A1 | 9/2014  | Xu et al.        |
| 2011/0094406 A1 | 4/2011  | Marya et al.             | 2014/0360728 A1 | 12/2014 | Tashiro et al.   |
| 2011/0100643 A1 | 5/2011  | Themig et al.            | 2015/0060085 A1 | 3/2015  | Xu               |
| 2011/0127044 A1 | 6/2011  | Radford et al.           | 2015/0065401 A1 | 3/2015  | Xu et al.        |
| 2011/0132143 A1 | 6/2011  | Xu et al.                | 2016/0209391 A1 | 7/2016  | Zhang et al.     |
| 2011/0132612 A1 | 6/2011  | Agrawal et al.           | 2016/0258242 A1 | 9/2016  | Hayter et al.    |
| 2011/0132619 A1 | 6/2011  | Agrawal et al.           |                 |         |                  |
| 2011/0132620 A1 | 6/2011  | Agrawal et al.           |                 |         |                  |
| 2011/0132621 A1 | 6/2011  | Agrawal et al.           |                 |         |                  |
| 2011/0135530 A1 | 6/2011  | Xu et al.                |                 |         |                  |
| 2011/0135805 A1 | 6/2011  | Doucet et al.            |                 |         |                  |
| 2011/0135953 A1 | 6/2011  | Xu et al.                |                 |         |                  |
| 2011/0136707 A1 | 6/2011  | Xu et al.                |                 |         |                  |
| 2011/0139465 A1 | 6/2011  | Tibbles et al.           |                 |         |                  |
| 2011/0147014 A1 | 6/2011  | Chen et al.              |                 |         |                  |
| 2011/0186306 A1 | 8/2011  | Marya et al.             |                 |         |                  |
| 2011/0214881 A1 | 9/2011  | Newton et al.            |                 |         |                  |
| 2011/0247833 A1 | 10/2011 | Todd et al.              |                 |         |                  |
| 2011/0253387 A1 | 10/2011 | Ervin                    |                 |         |                  |
| 2011/0256356 A1 | 10/2011 | Tomantschger et al.      |                 |         |                  |
| 2011/0259610 A1 | 10/2011 | Shkurti et al.           |                 |         |                  |
| 2011/0277987 A1 | 11/2011 | Frazier                  |                 |         |                  |
| 2011/0277989 A1 | 11/2011 | Frazier                  |                 |         |                  |
| 2011/0284232 A1 | 11/2011 | Huang                    |                 |         |                  |
| 2011/0284240 A1 | 11/2011 | Chen et al.              |                 |         |                  |
| 2011/0284243 A1 | 11/2011 | Frazier                  |                 |         |                  |
| 2011/0300403 A1 | 12/2011 | Vecchio et al.           |                 |         |                  |
| 2011/0314881 A1 | 12/2011 | Hatcher et al.           |                 |         |                  |
| 2012/0024109 A1 | 2/2012  | Xu et al.                |                 |         |                  |
| 2012/0067426 A1 | 3/2012  | Soni et al.              |                 |         |                  |
| 2012/0090839 A1 | 4/2012  | Rudic                    |                 |         |                  |
| 2012/0103135 A1 | 5/2012  | Xu et al.                |                 |         |                  |
| 2012/0107590 A1 | 5/2012  | Xu et al.                |                 |         |                  |
| 2012/0118583 A1 | 5/2012  | Johnson et al.           |                 |         |                  |
| 2012/0130470 A1 | 5/2012  | Agnew et al.             |                 |         |                  |
| 2012/0145378 A1 | 6/2012  | Frazier et al.           |                 |         |                  |

## FOREIGN PATENT DOCUMENTS

|    |               |         |
|----|---------------|---------|
| CN | 1255879       | 6/2000  |
| CN | 2658384 Y     | 11/2004 |
| CN | 1668545 A     | 9/2005  |
| CN | 1882759 A1    | 12/2006 |
| CN | 101050417 A   | 10/2007 |
| CN | 101351523 A   | 1/2009  |
| CN | 101454074 A   | 6/2009  |
| CN | 101605963     | 12/2009 |
| CN | 101457321 B   | 6/2010  |
| CN | 101720378 A   | 6/2010  |
| EA | 008390 B1     | 4/2007  |
| EA | 200870227 A1  | 2/2009  |
| EP | 0033625 A1    | 8/1981  |
| EP | 1006258 A2    | 6/2000  |
| EP | 1174385 A2    | 1/2002  |
| EP | 1412175 B1    | 4/2004  |
| EP | 1798301 A1    | 8/2006  |
| EP | 1857570       | 11/2007 |
| FR | 2782096 A1    | 2/2000  |
| GB | 912956        | 12/1962 |
| GB | 1046330 A     | 10/1966 |
| GB | 1280833 A     | 7/1972  |
| GB | 1357065 A     | 6/1974  |
| JP | 6106770       | 4/1986  |
| JP | 7-54008       | 2/1995  |
| JP | 754008 A      | 2/1995  |
| JP | 08232029      | 9/1996  |
| JP | 08-232029     | 10/1996 |
| JP | 2000185725 A1 | 7/2000  |
| JP | 2002053902 A  | 2/2002  |
| JP | 2004225084    | 8/2004  |

(56)

## References Cited

## FOREIGN PATENT DOCUMENTS

|    |              |    |         |
|----|--------------|----|---------|
| JP | 2004225765   | A  | 8/2004  |
| JP | 2005076052   | A  | 3/2005  |
| JP | 2009144207   | A  | 7/2009  |
| JP | 2010502840   | A  | 1/2010  |
| KR | 95-0014350   |    | 11/1995 |
| RU | 2373375      | C2 | 11/2009 |
| WO | 9909227      | A1 | 2/1999  |
| WO | 9947726      |    | 9/1999  |
| WO | 03008186     | A1 | 1/2003  |
| WO | 2004001087   | A1 | 12/2003 |
| WO | 2004073889   | A1 | 9/2004  |
| WO | 2005040068   | A  | 5/2005  |
| WO | 2007044635   | A  | 4/2007  |
| WO | 2007095376   | A2 | 8/2007  |
| WO | 2008034042   | A3 | 3/2008  |
| WO | 2008/057045  | A1 | 5/2008  |
| WO | 2008079777   | A3 | 7/2008  |
| WO | WO2008079485 |    | 7/2008  |
| WO | 2009079745   | A1 | 7/2009  |
| WO | 2010012184   | A1 | 2/2010  |
| WO | 2011071902   | A3 | 6/2011  |
| WO | 2011071907   | A2 | 6/2011  |
| WO | 2011071910   | A2 | 6/2011  |
| WO | 2011071910   | A3 | 6/2011  |
| WO | 2011130063   | A3 | 2/2012  |
| WO | 2012015567   | A2 | 2/2012  |
| WO | 2012149007   | A2 | 11/2012 |
| WO | 2012164236   | A1 | 12/2012 |
| WO | 2012174101   | A2 | 12/2012 |
| WO | 2013053057   | A1 | 4/2013  |
| WO | 2013078031   | A1 | 5/2013  |
| WO | 2014121384   | A1 | 8/2014  |

## OTHER PUBLICATIONS

- CH. Christoglou, N. Voudouris, G.N. Angelopoulos, M. Pant, W. Dahl, "Deposition of Aluminum on Magnesium by a CVD Process", Surface and Coatings Technology 184 (2004) 149-155.
- Constantin Vahlas, Bri Gitte Caussat, Philippe Serp, George N. Angelopoulos, "Principles and Applications of CVD Powder Technology", Materials Sciene and Engineering R 53 (2006) 1-72.
- Guan Ling Song, Andrej Atrens "Corrosion Mechanisms of Magnesium Alloys", Advanced Engineering Materials 1999, 1, No. 1, pp. 11-33.
- H. Hermawan, H. Alamdar, D. Mantovani and Dominique Dube, "Iron-manganese: new class of metallic degradable biomaterials prepared by powder metallurgy", Powder Metallurgy, vol. 51, No. 1, (2008), pp. 38-45.
- J. Dutta Majumdar, B. Ramesh Chandra, B.L. Mordike, R. Galun, I. Manna, "Laser Surface Engineering of a Magnesium Alloy with Al + Al<sub>2</sub>O<sub>3</sub>", Surface and Cotaings Technology 179 (2004) 297-305.
- J.E. Gray, B. Luan, "Protective Coatings on Magnesuim and Its Alloys—A Critical Review", Journal of Alloys and Compounds 336 (2002) 88-113.
- Yihua Zhu, Chunzhong Li, Qiufang Wu, "The process of coating on ultrafine particles by surface hydrolysis reaction in a fluidized bed reactor", Surface and Coatings Technology 135 (2000) 14-17.
- Yi Feng, Hailong Yuan, "Electroless Plating of Carbon Nanotubes with Silver" Journal of Materials Science, 39, (2004) pp. 3241-3243.
- E Flahaut et al., "Carbon Nanotube-Metal-Oxide Nanocomposites: Microstructure, Electrical Conductivity and Mechanical Properties" Acta mater. 48 (2000) 3803-3812.
- C.S. Goh, J. Wei, L C Lee, and M. Gupta, "Development of novel carbon nanotube reinforced magnesium nanocomposites using the powder metallurgy technique", Nanotechnology 17 (2006) 7-12.
- Toru Kuzumaki, Osamu Ujiie, Hideki Ichinose, and Kunio Ito, "Mechanical Characteristics and Preparation of Carbon Nanotube Fiber-Reinforced Ti Composite", Advanced Engineering Materials, 2000, 2, No. 7.
- Shimizu et al., "Multi-walled carbon nanotube-reinforced magnesium alloy composites", Scripta Materialia, vol. 58, Issue 4, pp. 267-270.
- Jing Sun, Lian Gao, Wei Li, "Colloidal Processing of Carbon NanotubeAlumina Composites" Chem. Mater. 2002, 14, 5169-5172.
- Xiaotong Wang et al., "Contact-Damage-Resistant Ceramic/Single-Wall Carbon Nanotubes and Ceramic/Graphite Composites" Nature Materials, vol. 3, Aug. 2004, pp. 539-544.
- Y. Zhang and Hongjie Dai, "Formation of metal nanowires on suspended single-walled carbon nanotubes" Applied Physics Letter, vol. 77, No. 19 (2000), pp. 3015-3017.
- Guo-Dong Zhan, Joshua D. Kuntz, Julin Wan and Amiya K. Mukherjee, "Single-wall carbon nanotubes as attractive toughening agents in alumina-based nanocomposites" Nature Materials, vol. 2., Jan. 2003. 38-42.
- Y. Zhang, Nathan W. Franklin, Robert J. Chen, Hongjie Dai, "Metal Coating on Suspended Carbon Nanotubes and its Implication to Metal—Tube Interaction", Chemical Physics Letters 331 (2000) 35-41.
- Notification of Transmittal of the International Search Report and the Written Opinion of the International Searching Authority; PCT/US2011/047000; Korean Intellectual Property Office; Mailed Dec. 26, 2011; 8 pages.
- Flow Control Systems, [online]; [retrieved on May 20, 2010]; retrieved from the Internet <http://www.bakerhughes.com/products-and-services/completions-and-productions/well-completions/packers-and-flow-control/flow-control-systems>.
- Optisleeve Sliding Sleeve, [online]; [retrieved on Jun. 25, 2010]; retrieved from the Internet [weatherfordcorp/WFT033159.pdf](http://weatherford.com/weatherford/groups/.../weatherfordcorp/WFT033159.pdf).
- "Sliding Sleeve", Omega Completion Technology Ltd, Sep. 29, 2009, retrieved on: [www.omega-completion.com](http://www.omega-completion.com).
- Welch, William R. et al., "Nonelastomeric Sliding Sleeve Maintains Long Term Integrity in HP/HT Application: Case Histories." [Abstract Only], SPE Eastern Regional Meeting, Oct. 23-25, 1996, Columbus, Ohio.
- Notification of Transmittal of the International Search Report and the Written Opinion of the International Searching Authority, or the Declaration mailed on Feb. 23, 2012 (Dated Feb. 22, 2012) for PCT/US2011/043036.
- International Search Report and Written Opinion of the International Searching Authority, or the Declaration for PCT/US2011/058105 mailed from the Korean Intellectual Property Office on May 1, 2012.
- International Search Report and Written Opinion of the International Searching Authority for International Application No. PCT/US2011/058099 (filed on Oct. 27, 2011), mailed on May 11, 2012.
- Baker Hughes Tools. "Baker Oil Tools Introduces Revolutionary Sand Control Completion Technology," May 2, 2005.
- E. Paul Bercegeay et al., "A One-Trip Gravel Packing System"; Society of Petroleum Engineers, Offshore Technology Conference, SPE Paper No. 4771; Feb. 7-8, 1974.
- Bybee, Karen. "One-Trip Completion System Eliminates Perforations," Completions Today, Sep. 2007, pp. 52-53.
- Curtin, William and Brian Sheldon. "CNT-reinforced ceramics and metals," Materials Today, 2004, vol. 7, 44-49.
- Galanty et al. "Consolidation of metal powders during the extrusion process," Journal of Materials Processing Technology (2002), pp. 491-496.
- Hjortstam et al. "Can we achieve ultra-low resistivity in carbon nanotube-based metal composites," Applied Physics A (2004), vol. 78, Issue 8, pp. 1175-1179.
- Notification of Transmittal of the International Search Report and the Written Opinion of the International Searching Authority; PCT/US2010/059259; International Searching Authority KIPO; Mailed Jun. 13, 2011.
- Notification of Transmittal of the International Search Report and the Written Opinion of the International Searching Authority; PCT/US2010/059265; International Searching Authority KIPO; Mailed Jun. 16, 2011.

(56)

## References Cited

## OTHER PUBLICATIONS

- Notification of Transmittal of the International Search Report and the Written Opinion of the International Searching Authority; PCT/US2010/059268; International Searching Authority KIPO; Mailed Jun. 17, 2011.
- Stephen P. Mathis, "Sand Management: A Review of Approaches and Concerns"; Society of Petroleum Engineers, SPE Paper No. 82240; SPE European Formation Damage Conference, The Hague, The Netherlands, May 13-14, 2003.
- Pardo, et al.; "Corrosion Behaviour of Magnesium/Aluminium Alloys in 3.5 wt% NaCl"; Corrosion Science; 50; pp. 823-834; (2008).
- Notification of Transmittal of the International Search Report and Written Opinion, Mailed Jul. 8, 2011, International Appln. No. PCT/US2010/059263, Written Opinion 4 Pages, International Search Report 3 Pages.
- Song, G. and S. Song. "A Possible Biodegradable Magnesium Implant Material," Advanced Engineering Materials, vol. 9, Issue 4, Apr. 2007, pp. 298-302.
- Song, et al.; "Understanding Magnesium Corrosion"; Advanced Engineering Materials; 5; No. 12; pp. 837-858; (2003).
- Zeng et al. "Progress and Challenge for Magnesium Alloys as Biomaterials," Advanced Engineering Materials, vol. 10, Issue 8, Aug. 2008, pp. B3-B14.
- Ambat, et al.; "Electroless Nickel-Plating on AZ91D Magnesium Alloy: Effect of Substrate Microstructure and Plating Parameters"; Surface and Coatings Technology; 179; pp. 124-134; (2004).
- Chang, et al.; "Electrodeposition of Aluminum on Magnesium Alloy in Aluminum Chloride (AlCl<sub>3</sub>)-1-ethyl-3- methylimidazolium chloride (EMIC) Ionic Liquid and Its Corrosion Behavior"; Electrochemistry Communications; 9; pp. 1602-1606; (2007).
- Forsyth, et al.; "An Ionic Liquid Surface Treatment for Corrosion Protection of Magnesium Alloy AZ31"; Electrochem. Solid-State Lett./ 9(11); 4 pages.
- Forsyth, et al.; "Exploring Corrosion Protection of Mg Via Ionic Liquid Pretreatment"; Surface & Coatings Technology; 201; pp. 4496-4504; (2007).
- Hsiao et al.; "Effect of Heat Treatment on Anodization and Electrochemical Behavior of AZ91D Magnesium Alloy"; J. Mater. Res.; 20(10); pp. 2763-2771; (2005).
- Hsiao, et al.; "Anodization of AZ91D Magnesium Alloy in Silicate-Containing Electrolytes"; Surface & Coatings Technology; 199; pp. 127-134; (2005).
- Hsiao, et al.; "Baking Treatment Effect on Materials Characteristics and Electrochemical Behavior of anodic Film Formed on AZ91D Magnesium Alloy"; Corrosion Science; 49; pp. 781-793; (2007).
- Hsiao, et al.; "Characterization of Anodic Films Formed on AZ91D Magnesium Alloy"; Surface & Coatings Technology; 190; pp. 299-308; (2005).
- Huo et al.; "Corrosion of AZ91D Magnesium Alloy with a Chemical Conversion Coating and Electroless Nickel Layer"; Corrosion Science; 46; pp. 1467-1477; (2004).
- Liu, et al.; "Electroless Nickel Plating on AZ91 Mg Alloy Substrate"; Surface & Coatings Technology; 200; pp. 5087-5093; (2006).
- Lunder et al.; "The Role of Mg<sub>17</sub>Al<sub>12</sub> Phase in the Corrosion of Mg Alloy AZ91"; Corrosion; 45(9); pp. 741-748; (1989).
- Shi et al.; "Influence of the Beta Phase on the Corrosion Performance of Anodised Coatings on Magnesium-Aluminium Alloys"; Corrosion Science; 47; pp. 2760-2777; (2005).
- Song, et al.; "Corrosion Mechanisms of Magnesium Alloys"; Advanced Engineering Materials; 1(1); pp. 11-33; (1999).
- Song, Guangling; "Recent Progress in Corrosion and Protection of Magnesium Alloys"; Advanced Engineering Materials; 7(7); pp. 563-586; (2005).
- Song, et al.; "Influence of Microstructure on the Corrosion of Diecast AZ91D"; Corrosion Science; 41; pp. 249-273; (1999).
- Song, et al.; "Corrosion Behaviour of AZ21, AZ501 and AZ91 in Sodium Chloride"; Corrosion Science; 40(10); pp. 1769-1791; (1998).
- Zhang, et al; "Study on the Environmentally Friendly Anodizing of AZ91D Magnesium Alloy"; Surface and Coatings Technology; 161; pp. 36-43; (2002).
- International Search Report and Written Opinion; Mail Date Jul. 28, 2011; International Application No. PCT/US2010/057763; International Filing date Nov. 23, 2010; Korean Intellectual Property Office; International Search Report 7 pages; Written Opinion 3 pages.
- Patent Cooperation Treaty International Search Report and Written Opinion for International Patent Application No. PCT/US2012/034978 filed on Apr. 25, 2012, mailed on Nov. 12, 2012.
- Canadian Pat. App. No. 2783241 filed on Dec. 7, 2010, published on Jun. 16, 2011 for "Nanomatrix Powder Metal Compact".
- Canadian Pat. App. No. 2783346 filed on Dec. 7, 2010, published on Jun. 16, 2011 for "Engineered Powder Compact Composite Material".
- International Search Report and Written Opinion for International application No. PCT/US20121034973 filed on Apr. 25, 2012, mailed on Nov. 29, 2012.
- Wikipedia, the free encyclopedia. Reactivity series. [http://en.wikipedia.org/w/index.php?title=Reactivity\\_series&printable=yes](http://en.wikipedia.org/w/index.php?title=Reactivity_series&printable=yes) downloaded on May 18, 2014. 8 pages.
- Constantine, Jesse. "Selective Production of Horizontal Openhole Completions Using ECP and Sliding Sleeve Technology." SPE Rocky Mountain Regional Meeting, May 15-18, 1999, Gillette, Wyoming. [Abstract Only].
- E.J. Lavenia, B.Q. Han, J.M. Schoenung; "Cryomilled nanostructured materials: Processing and properties", Materials Science and Engineering A, 493, (2008) 207-214.
- Elsayed Ayman, Imai Hisashi, Umeda Junko and Kondoh Katsuyoshi, "Effect of Consolidation and Extrusion Temperatures on Tensile Properties of Hot Extruded ZK61 Magnesium Alloy Gas Atomized Powders via Spark Plasma Sintering" Transaction of JWRI, vol. 38, (2009) No. 2, pp. 31-35.
- H. Watarai, Trend of research and development for magnesium alloys-reducing the weight of structural materials in motor vehicles, (2006) Science and technology trends, Quarterly review No. 18, 84-97.
- Bing Q. Han, Enrique J. Lavernia and Farghali A. Mohamed, "Mechanical Properties of Nanostructured Materials", Rev. Adv. Mater. Sci. 9(2005) 1-16.
- International Search Report and Written Opinion, International Application No. PCT/US2012/049434, Date of Mailing Feb. 1, 2013, Korean Intellectual Property Office, Written Opinion 4 pages, International Search Report 3 pages.
- International Search Report and Written Opinion for PCT Application No. PCT/US2012/044866, dated Jan. 2, 2013, pp. 1-9.
- International Search Report and Written Opinion, PCT/US2012/046231, Date of Mailing Jan. 29, 2013, Korean Intellectual Property Office, Written Opinion 6 pages, International Search Report 3 pages.
- M. Bououdina, Z. X. Guo, Comparative study of mechanical alloying of (Mg+Al) and (Mg+Al+Ni) mixtures for hydrogen storage, J. Alloys, Compds, 2002, 336, 222-231.
- M.Liu, P.J. Uggowitzer, A.V. Nagasekhar, P. Schmutz, M. Easton, G.L. Song, A. Atrens, Calculated phase diagrams and the corrosion of die-cast Mg—Al alloys, Corrosion Science, 2009, 51, 606-619.
- Adam J. Maisano, "Cryomilling of Aluminum-Based and Magnesium-Based Metal Powders", Thesis, Virginia Tech, Jan. 13, 2006.
- International Search Report and Written Opinion; PCT/US2010/059257; Korean Intellectual Property Office; dated Jul. 27, 2011.
- International Search Report and Written Opinion; PCT/US2012/038622; Dated Dec. 6, 2012; 12 pages.
- S.L. Lee, C.W. Hsu, F.K. Hsu, C.Y. Chou, C.K. Lin, C.W. Weng, Effects of Ni addition on hydrogen storage properties of Mg<sub>17</sub>Al<sub>12</sub> alloy, Materials Chemistry and Physics, 2011, 126, 319-324.
- Shumbera et al. "Improved Water Injector Performance in a Gulf of Mexico Deepwater Development Using an Openhole Frac Pack Completion and Downhole Filter System: Case History." SPE Annual Technical Conference and Exhibition, Oct. 5-8, 2003, Denver, Colorado. [Abstract Only].

(56)

## References Cited

## OTHER PUBLICATIONS

- T.J. Bastow, S. Celotto, Clustering and formation of nano-precipitates in dilute aluminum and magnesium alloys, *Materials science and Engineering*, 2003, C23, 757-762.
- Vickery, Harold and Christian Bayne, "New One-Trip Multi-Zone Frac Pack System with Positive Positioning." European Petroleum Conference, Oct. 29-31, 2002, Aberdeen, UK. [Abstract Only].
- H. Watanabe, T. Mukai, M. Mabuchi and K. Higashi, "Superplastic Deformation Mechanism in Powder Metallurgy Magnesium Alloys and Composites", *Acta mater.* 49 (2001) pp. 2027-2037.
- Xiaowu Nie, Patents of Methods to Prepare Intermetallic Matrix Composites: A Review, *Recent Patents on Materials Science* 2008, 1, 232-240, Department of Scientific Research, Hunan Railway College of Science and Technology, Zhuzhou, P.R. China.
- Baker Oil Tools. "Z-Seal Metal-to-Metal Expandable Sealing Device Uses Expanding Metal in Place of Elastomers," Nov. 6, 2006.
- Baker Hughes Incorporated. IN-Tallic Disintegrating Frac Balls. Houston: Baker Hughes Incorporated, 2011. Accessed Mar. 6, 2015.
- Baker Hughes, "Multistage", Oct. 31, 2011, BakerHughes.com; accessed Mar. 6, 2015.
- International Search Report and Written Opinion; International Application No. PCT/US2012/071742; International Filing Date: Dec. 27, 2012; Date of Mailing: Apr. 22, 2013; 12 pages.
- International Search Report and Written Opinion; International Application No. PCT/US2014/058997, International Filing Date: Oct. 3, 2014; Date of Mailing: Jan. 12, 2015; 12 pages.
- International Search Report; International Application No. PCT/US2012/044229, International Filing Date: Jun. 26, 2012; Date of Mailing: Jan. 30, 2013; 3 pages.
- Murray, "Binary Alloy Phase Diagrams" *Int. Met. Rev.*, 30(5) 1985 vol. 1, pp. 103-187.
- Vernon Constien et al., "Development of Reactive Coatings to Protect Sand-Control Screens", SPE 112494, Copyright 2008, Society of Petroleum Engineers, This paper was prepared for presentation at the 2008 SPE International Symposium and Exhibition on for.
- "Reactivity series", Wikipedia, [http://en.wikipedia.org/w/index.php?title=Reactivity\\_series&printable=yes](http://en.wikipedia.org/w/index.php?title=Reactivity_series&printable=yes) downloaded on May 18, 2014. 8 pages.
- Adams, et al.; "Thermal stabilities of aromatic acids as geothermal tracers", *Geothermics*, vol. 21, No. 3, 1992, pp. 323-339.
- Ayman, et al.; "Effect of Consolidation and Extrusion Temperatures on Tensile Properties of Hot Extruded ZK61 Magnesium Alloy Gas Atomized Powders via Spark Plasma Sintering", *Transactions of JWRI*, vol. 38 (2009), No. 2, pp. 1-5.
- Bastow, et al., "Clustering and formation of nano-precipitates in dilute aluminum and magnesium alloys", *Materials Science and Engineering*, 2003, C23, 757-762.
- Birbilis, et al., "Exploring Corrosion Protection of Mg Via Ionic Liquid Pretreatment", *Surface & Coatings Technology*; 201, pp. 4496-4504, (2007).
- Carrejo, et al., "Improving Flow Assurance in Multi-Zone Fracturing Treatments in Hydrocarbon Reservoirs with High Strength Corrodible Tripping Balls"; Society of Petroleum Engineers; SPE Paper No. 151613; Apr. 16, 2012; 6 pages.
- Feng, et al., "Electroless Plating of Carbon Nanotubes with Silver" *Journal of Materials Science*, 39, (2004) pp. 3241-3243.
- Flahaut, et al., "Carbon Nanotube-Metal-Oxide Nanocomposites: Microstructure, Electrical Conductivity and Mechanical Properties" *Acta mater.* 48 (2000), pp. 3803-3812.
- Garfield, New One-Trip Sand-Control Completion System that Eliminates Formation Damage Resulting From conventional Perforating and Gravel-Pack Operations; SPE Annual Technical Conference and Exhibition, Oct. 9-12, 2005.
- Garfield, et al., "Maximizing Inflow Performance in Soft Sand Completions Using New One-trip Sand Control Liner Completion Technology", SPE European Formation Damage Conference, May 25-27, 2005.
- Goh, et al., "Development of novel carbon nanotube reinforced magnesium nanocomposites using the powder metallurgy technique", *Nanotechnology* 17 (2006) 7-12.
- International Search Report and Written Opinion; International Application No. PCT/US2012/038622; International Filing Date: May 18, 2012; Date of Mailing: Dec. 6, 2012; 12 pages.
- International Search Report and Written Opinion; International Application No. PCT/US2012/049434; International Filing Date: Aug. 3, 2012; Date of Mailing: Feb. 1, 2013; 7 pages.
- International Search Report and Written Opinion; International Application No. PCT/US2012/053339; International Filing Date: Aug. 31, 2012; Date of Mailing: Feb. 15, 2013; 11 pages.
- International Search Report and Written Opinion; International Application No. PCT/US2012/053342; International Filing Date: Aug. 31, 2012; Date of Mailing: Feb. 19, 2013; 9 pages.
- International Search Report and Written Opinion; International Application No. PCT/US2012/053350; International Filing Date: Aug. 31, 2012; Date of Mailing: Feb. 25, 2013; 10 pages.
- International Search Report and Written Opinion; International Application No. PCT/US2014/049347; International Filing Date: Aug. 1, 2014; Date of Mailing: Nov. 24, 2014; 11 pages.
- International Search Report and Written Opinion; International Application No. PCT/US2014/054720; International Filing Date: Sep. 9, 2014; Date of Mailing: Dec. 17, 2014; 10 pages.
- Li, et al. "Investigation of aluminium-based nanocomposites with ultra-high strength", *Materials Science and Engineering A*, 527, pp. 305-316, (2009).
- Mathis, "Sand Management: A Review of Approaches and Concerns", Society of Petroleum Engineers, SPE Paper No. 82240, SPE European Formation Damage Conference, the Hague, the Netherlands, May 13-14, 2003.
- Nie, "Patents of Methods to Prepare Intermetallic Matrix Composites: A Review", *Recent Patents on Materials Science* 2008, vol. 1, pp. 232-240.
- Rose, et al.; "The application of the polyaromatic sulfonates as tracers in geothermal reservoirs", *Geothermics* 30 (2001) pp. 617-640.
- Seyni, et al., "On the interest of using degradable fillers in co-ground composite materials", *Powder Technology* 190, (2009) pp. 176-184.
- Shaw, "Benefits and Application of a Surface-Controlled Sliding Sleeve for Fracturing Operations"; Society of Petroleum Engineers, SPE Paper No. 147546; Oct. 30, 2011; 8 pages.
- Shigematsu, et al., "Surface Treatment of AZ91D Magnesium Alloy by Aluminum diffusion Coating", *Journal of Materials Science Letters* 19, 2000, pp. 473-475.
- Singh, et al., "Extended Homogeneity Range of Intermetallic Phases in Mechanically Alloyed Mg-Al Alloys", Elsevier Sciences Ltd., *Intermetallics* 11, 2003, pp. 373-376.
- Stanley, et al.; "An Introduction to Ground-Water Tracers", Department of Hydrology and Water Resources, University of Arizona, Mar. 1985, pp. 1-219.
- Sun, et al.; "Colloidal Processing of Carbon Nanotube/Alumina Composites" *Chem. Mater.* 2002, 14, pp. 5169-5172.
- Walters, et al.; "A Study of Jets from Unsintered-Powder Metal Lined Nonprecision Small-Caliber Shaped Charges", Army Research Laboratory, Aberdeen Proving Ground, MD 21005-5066; Feb. 2001.
- Xu, et al., "Nanostructured Material-Based Completion Tools Enhance Well Productivity"; International Petroleum Technology Conference; Conference Paper IPTC 16538; International Petroleum Technology Conference 2013; 4 pages.
- Zemel, "Tracers in the Oil Field", University of Texas at Austin, Center for Petroleum and Geosystems, Jan. 1995, Chapters 1, 2, 3, 7.
- Zhang, et al.; "High Strength Nanostructured Materials and Their Oil Field Applications"; Society of Petroleum Engineers; Conference Paper SPE 157092; SPE International Oilfield Nanotechnology Conference, 2012; 6 pages.
- Aviles et al, "Degradable Alternative to Risky Mill-Out Operations in Plug and Per"; SPE-173695-MS; Society of Petroleum Engineers; SPE/ICOTA Coiled Tubing & Well Intervention Conference & Exhibition; Mar. 24-25, 2015; 10 Pages.

(56)

**References Cited****OTHER PUBLICATIONS**

- Bin et al., "Advances in Fluidization CVD Technology", East China University of Chemical Technology, China Academic Journal Electronic Publishing House, vol. 13, No. 4, Nov. 1992, pp. 360-365, English Abstract on p. 366.
- Garry Garfield, "Formation Damage Control Utilizing Composite-Bridge-Plug Technology for Monobore, Multizone Stimulation Operations," SPE 70004, 2001, Society of Petroleum Engineers Inc.. This paper was prepared for presentation at the SPE Per. International Preliminary Report on Patentability; PCT/US2013/050475; Mailed Feb. 26, 2015; 10 Pages.
- International Search Report and Written Opinion, Date of Mailing Feb. 26, 2013; International Application No. PCT/US2012/047163, Korean Intellectual Property Office; Written Opinion 9 pages, International Search Report 3 pages.
- International Search Report and Written Opinion; International Application No. PCT/US2012/052836; International Filing Date: Aug. 29, 2012; Date of Mailing Feb. 1, 2013; 9 pages.
- International Search Report for related PCT Application No. PCT/US2013/035258, dated Jul. 4, 2013, pp. 1-4.
- International Search Report for related PCT Application No. PCT/US2013/035261, dated Jul. 10, 2013, pp. 1-4.
- International Search Report for related PCT Application No. PCT/US2013/035262, dated Jul. 1, 2013, pp. 1-4.
- International Search Report for related PCT Application No. PCT/US2013/068062, dated Feb. 12, 2014, pp. 1-3.
- Lin et al., "Processing and Microstructure of Nano-Mo/Al<sub>2</sub>O<sub>3</sub> Composites from Mocvd and Fluidized Bed", Nanostructured Materials, Nov. 1999, vol. 11, No. 8, pp. 1361-1377.
- M.S. Senthil Saravanan et al., "Mechanically Alloyed Carbon Nanotubes (CNT) Reinforced Nanocrystalline AA 4032: Synthesis and Characterization," Journal of Minerals & Materials Characterization & Engineering, vol. 9, No. 11, pp. 1027-1035, 2010.
- M.T. Triolo et al., "Resolving the Completion Engineer's Dilemma: Permanent or Retrievable Packer?", Society of Petroleum Engineers, SPE Paper No. 76711; May 20, 2002; 16 pages.
- Martin P. Coronado, "Development of an Internal Coiled Tubing Connector Utilizing Permanent Packer Technology"; Society of Petroleum Engineers, SPE Paper No. 46036; Apr. 15, 1998; 10 pages.
- Notification of Transmittal of the International Search Report and the Written Opinion of the International Searching Authority, or the Declaration; PCT/US2014/010862; 21 Apr. 2014; 9 pages.
- Notification of Transmittal of the International Search Report on Patentability and the Written Opinion of the International Searching Authority, or the Declaration; PCT/US2013/020046; Apr. 10, 2013, 7 pages.
- Quik Drill Composite Frac Plug; Baker Hughes, Baker Oil Tools; Copyright 2002; 3 pages.
- S.R. Bakshi et al., "Carbon nanotube reinforced metal matrix composites—a review," International Materials Reviews; 2010, pp. 41-64, vol. 55, No. 1.
- Simulia Realistic Simulation News, [online]; [retrieved on Jan. 10, 2013]; retrieved from the internet [http://www.3ds.com/fileadmin/brands/SIMULIA/Customer\\_Stories/Baker\\_Hughes/Energy\\_BakerHughes\\_RSN\\_Feb11.pdf](http://www.3ds.com/fileadmin/brands/SIMULIA/Customer_Stories/Baker_Hughes/Energy_BakerHughes_RSN_Feb11.pdf), Baker Hughes Refines Expandable Tubular.
- Spencer et al., "Fluidized Bed Polymer Particle ALD Process for Producing Hdpe/Alumina Nanocomposites" in "The 12th International Conference on Fluidization—New Horizons in Fluidization Engineering" [ . . . ] vol. RP4 (2007).
- Australian Examination Report for Australian patent application No. 2012302067 dated Sep. 22, 2015.
- Australian Examination Report; Australian Application No. 2012287461; Date of Mailing: Jul. 13, 2015; 6 pages.
- Aviles et al, "Degradable Alternative to Risky Mill-Out Operations in Plug and Perf"; SPE-173695-MS; Society of Petroleum Engineers; SPE/ICOTA Coiled Tubing & Well Intervention Conference & Exhibition; Mar. 15-18, 2015; 10 Pages.
- Chinese Office Action for Chinese Application No. 201280036477. 4, dated Nov. 4, 2015, pp. 1-15.
- Chinese Office Action; Chinese Application No. 201280020572.5; Mailing Date:Oct. 10, 2015; 13 pages.
- Chuan-Jun et al., "Study on Corrosion Kinetics of Mg—Ni alloys", Journal of Kunming University of Science and Technology, vol. 34, No. 5, pp. 10-13, Oct. 2009.
- European Search Report for EP Application No. 10836533.9 dated Jul. 27, 2015.
- European Search Report for EP Application No. 10836538.8 dated Jul. 27, 2015.
- European Search Report for EP Application No. 10836539.6 dated Jul. 27, 2015.
- European Search Report for EP Application No. 10836540.4 dated Aug. 20, 2015.
- International Search Report for related PCT Application No. PCT/US2013/1035258, dated Jul. 4, 2013, pp. 1-4.
- International Search Report for related PCT Application No. PCT/US2013/1035261, dated Jul. 10, 2013, pp. 1-4.
- International Search Report for related PCT Application No. PCT/US2013/1035262, dated Jul. 1, 2013, pp. 1-4.
- International Search Report for related PCT Application No. PCT/US2013/1068062, dated Feb. 12, 2014, pp. 1-3.
- Tsipas et al. "Effect of High Energy Ball Milling on Titanium-Hydroxyapatite Powders" Powder Metallurgy, Maney Publishing, London, GB, vol. 46, No. 1, Mar. 2003 (Mar. 2003), pp. 73-77.
- Australian Office Action for Patent Application No. 2012302067; Date of Issue Feb. 2, 2015, 3 pages.
- Australian Patent Examination Report for Patent Application No. 2012302067 dated Sep. 22, 2015, 3 pages.
- Canadian Office Action for Application No. 2860699; Date of Mailing Oct. 7, 2015, 4 pages.
- Canadian Office Action for Canadian Application No. 2,841,068, dated Nov. 9, 2015, pp. 14.
- Chinese Office Action for Chinese Application No. 201280041320. 0; Date of Mailing Jun. 6, 2016, 14 pages.
- Chinese Office Action for Chinese Application No. 201380006291.9 dated Apr. 27, 2016, 25 pages.
- Chinese Office Action for Chinese Patent Application No. 201280041531.4 dated Aug. 31, 2015.
- Office Action issued on Mar. 23, 2016 in related EP Patent Application No. 12827733.2.
- European Search Report for EP Application No. 12827733.2 dated Jan. 21, 2015; 6 pages.
- European Search Report for EP Application No. 12827915.5 dated Dec. 23, 2015; 8 pages.
- European Search Report for EP Application No. 12828903.0 dated Dec. 23, 2015.
- European Search Report for European Application No. 12820355. Jan. 1353, dated Dec. 18, 2015, 9 pages.
- Extended European Search Report for EP Application No. 12828379.3-1373, dated May 20, 2016, 8 pages.
- Extended European Search Report; EP Application No. 12822169A-1605/2739812; Mailing Date: Nov. 17, 2015; 14 pages.
- International Search Report and Written Opinion; International Application No. PCT/US2015/066353; International filing Date: Dec. 17, 2015; Date of Mailing: Apr. 1, 2016; 14 pages.
- M.S. Senthil Saravanan et al, "Mechanically Alloyed Carbon Nanotubes (CNT) Reinforced Vanocrystalline AA 4032: Synthesis and Characterization", Journal of Minerals and Materials Characterization and Engineering, vol. 9, No. 11 pp. 1027-1035 2010.
- Malaysian Search Report for Application No. PI 2012002545 dated May 31, 2016, 3 pages.
- Office Action issued on Feb. 1, 2016 in related Canadian Patent Application No. 2,844,517, 4 pages.
- Reid, Gary Carl, "Literature evaluation of induced groundwater tracers, field tracer techniques, and hydrodynamic dispersion values in porous media", Thesis in Geosciences (Masters), Texas Tech University, Aug. 1981, 109 pages.
- International Search Report and Written Opinion, International Application No. PCT/US2016/041849, Date of Mailing Oct. 26, 2016, Korean Intellectual Property Office; International Search Report 5 pages, Written Opinion 7 pages.

(56)

**References Cited**

OTHER PUBLICATIONS

- “Declaration of Karl T. Hartwig in Support of Petitioner Pursuant to 37 C.F.R. §42.120”, executed on Nov. 21, 2016 in support of U.S. Pat. No. 8,573,295, 52 pages.
- “Declaration of Karl T. Hartwig in Support of Petitioner Pursuant to 37 C.F.R. §42.120”, executed on Nov. 21, 2016 in support of U.S. Pat. No. 9,101,978, 51 pages.
- AP African Office Action for African Application No. AP/P/2014/007389, dated Oct. 6, 2016, 5 pages.
- Callister, Jr., William D., Materials Science and Engineering an Introduction, Seventh Edition, 2006, pp. 111, 627, and G7.
- German, Randall M., Powder Metallurgy Science, Second Edition, 1994, 102 pages.
- Klar, Erhard, ASM Handbook: International Metals Handbook—Powder Metallurgy, vol. 7, 1997, pp. 14, 276, and 798.
- Petition for Inter Partes Review; Case No. IPR2017-00326; U.S. Pat. No. 9,101,978; Nov. 23, 2016; 46 pages.
- Petition for Inter Partes Review; Case No. IPR2017-00327; U.S. Pat. No. 8,573,295; Nov. 23, 2016; 53 pages.
- Schaffer, James P. et al., The Science and Design of Engineering Materials, Second Edition, 1999, pp. 122, 123, 598, and 699.
- Kie, Guoqiang et al., “TEM Observation of Interfaces between Particles in Al-Mg Alloy Powder Compacts Prepared by Pulse Electric Current Sintering”, Materials Transactions, 2002, pp. 2177-2180, vol. 43-No. 9.
- Russian Search Report, Russian Application No. 2014149137, Date of Mailing Feb. 8, 2017; 4 pages.
- EP Search Report, PCT/US2012049434; Application No. EP 12823958; Date: Jun. 15, 2016; 9 pages.

\* cited by examiner



FIG. 1



FIG. 2



FIG. 3



FIG. 4



FIG. 5





FIG. 8



FIG. 9



FIG. 10



FIG. 15





FIG. 13



FIG. 14



FIG. 16



FIG. 17

| Material ID | Particle Core | Metallic Coating Layer<br>(e.g., 1 <sup>st</sup> +2 <sup>nd</sup> +3 <sup>rd</sup> ) |
|-------------|---------------|--------------------------------------------------------------------------------------|
| DHS1-1      | Mg            | No                                                                                   |
| DHS1-2      | Mg            | Al                                                                                   |
| DHS1-3      | Mg            | Ni + Al                                                                              |
| DHS1-4      | Mg            | W + Al                                                                               |
| DHS1-5      | Mg            | Al + Al <sub>2</sub> O <sub>3</sub> + Al                                             |
| DHS2-6      | Mg            | Al                                                                                   |

FIG. 18



FIG. 22



FIG. 19



FIG. 20



FIG. 21



FIG. 23



FIG. 24



FIG. 25

## 1

COATED METALLIC POWDER AND  
METHOD OF MAKING THE SAMECROSS REFERENCE TO RELATED  
APPLICATIONS

This application contains subject matter related to the subject matter of co-pending applications, which are assigned to the same assignee as this application, Baker Hughes Incorporated of Houston, Tex. and are all being filed on Dec. 8, 2009. The below listed applications are hereby incorporated by reference in their entirety:

U.S. patent application Ser. No. 12/633,682, entitled NANOMATRIX POWDER METAL COMPACT;

U.S. patent application Ser. No. 12/633,688, entitled METHOD OF MAKING A NANOMATRIX POWDER METAL COMPACT;

U.S. patent application Ser. No. 12/633,678, entitled ENGINEERED POWDER COMPACT COMPOSITE MATERIAL;

U.S. patent application Ser. No. 12/633,683, entitled TELESCOPIC UNIT WITH DISSOLVABLE BARRIER;

U.S. patent application Ser. No. 12/633,662 entitled DIS-SOLVING TOOL AND METHOD;

U.S. patent application Ser. No. 12/633,677 entitled MULTI-COMPONENT DISAPPEARING TRIPPING BALL AND METHOD FOR MAKING THE SAME; and

U.S. patent application Ser. No. 12/633,668 entitled DIS-SOLVING TOOL AND METHOD.

## BACKGROUND

Oil and natural gas wells often utilize wellbore components or tools that, due to their function, are only required to have limited service lives that are considerably less than the service life of the well. After a component or tool service function is complete, it must be removed or disposed of in order to recover the original size of the fluid pathway for use, including hydrocarbon production, CO<sub>2</sub> sequestration, etc. Disposal of components or tools has conventionally been done by milling or drilling the component or tool out of the wellbore, which are generally time consuming and expensive operations.

In order to eliminate the need for milling or drilling operations, the removal of components or tools by dissolution of degradable polylactic polymers using various wellbore fluids has been proposed. However, these polymers generally do not have the mechanical strength, fracture toughness and other mechanical properties necessary to perform the functions of wellbore components or tools over the operating temperature range of the wellbore, therefore, their application has been limited.

Other degradable materials have been proposed including certain degradable metal alloys formed from certain reactive metals in a major portion, such as aluminum, together with other alloy constituents in a minor portion, such as gallium, indium, bismuth, tin and mixtures and combinations thereof, and without excluding certain secondary alloying elements, such as zinc, copper, silver, cadmium, lead, and mixtures and combinations thereof. These materials may be formed by melting powders of the constituents and then solidifying the melt to form the alloy. They may also be formed using powder metallurgy by pressing, compacting, sintering and the like a powder mixture of a reactive metal and other alloy constituent in the amounts mentioned. These materials include many combinations that utilize metals, such as lead, cadmium, and the like that may not be suitable for release

## 2

into the environment in conjunction with the degradation of the material. Also, their formation may involve various melting phenomena that result in alloy structures that are dictated by the phase equilibria and solidification characteristics of the respective alloy constituents, and that may not result in optimal or desirable alloy microstructures, mechanical properties or dissolution characteristics.

Therefore, the development of materials that can be used to form wellbore components and tools having the mechanical properties necessary to perform their intended function and then removed from the wellbore by controlled dissolution using wellbore fluids is very desirable.

## SUMMARY

An exemplary embodiment of a metallic powder is disclosed. The metallic powder includes a plurality of metallic powder particles. Each powder particle includes a particle core. The particle core includes a core material comprising Mg, Al, Zn or Mn, or a combination thereof, having a melting temperature (T<sub>P</sub>). Each powder particle also includes a metallic coating layer disposed on the particle core. The metallic coating layer includes a metallic coating material having a melting temperature (T<sub>C</sub>). The powder particles are configured for solid-state sintering to one another at a predetermined sintering temperature (T<sub>S</sub>), and T<sub>S</sub> is less than T<sub>P</sub> and T<sub>C</sub>.

Another exemplary embodiment of a metallic powder is also disclosed. The metallic powder includes a plurality of metallic powder particles. Each powder particle includes a particle core. The particle core includes a core material comprising a metal having a standard oxidation potential less than Zn, ceramic, glass, or carbon, or a combination thereof, having a melting temperature (T<sub>P</sub>). Each powder particle also includes a metallic coating layer disposed on the particle core. The metallic coating layer includes a metallic coating material having a melting temperature (T<sub>C</sub>). The powder particles are configured for solid-state sintering to one another at a predetermined sintering temperature (T<sub>S</sub>), and T<sub>S</sub> is less than T<sub>P</sub> and T<sub>C</sub>.

Yet another exemplary embodiment includes a method of making a metallic powder. The method includes forming a metallic powder comprising a plurality of powder particles comprising Mg, Al, Zn or Mn, or a combination thereof, having a melting temperature (T<sub>P</sub>), for use as a plurality of particle cores. The method also includes depositing a metallic coating layer on each of the plurality of particle cores, the metallic coating layer having a melting temperature (T<sub>C</sub>), wherein the powder particles are configured for solid-state sintering to one another at a predetermined sintering temperature (T<sub>S</sub>), and T<sub>S</sub> is less than T<sub>P</sub> and T<sub>C</sub>.

## BRIEF DESCRIPTION OF THE DRAWINGS

Referring now to the drawings wherein like elements are numbered alike in the several Figures:

FIG. 1 is a photomicrograph of a powder 10 as disclosed herein that has been embedded in an epoxy specimen mounting material and sectioned;

FIG. 2 is a schematic illustration of an exemplary embodiment of a powder particle 12 as it would appear in an exemplary section view represented by section 2-2 of FIG. 1;

FIG. 3 is a schematic illustration of a second exemplary embodiment of a powder particle 12 as it would appear in a second exemplary section view represented by section 2-2 of FIG. 1;

FIG. 4 is a schematic illustration of a third exemplary embodiment of a powder particle 12 as it would appear in a third exemplary section view represented by section 2-2 of FIG. 1;

FIG. 5 is a schematic illustration of a fourth exemplary embodiment of a powder particle 12 as it would appear in a fourth exemplary section view represented by section 2-2 of FIG. 1;

FIG. 6 is a schematic illustration of a second exemplary embodiment of a powder as disclosed herein having a multi-modal distribution of particle sizes;

FIG. 7 is a schematic illustration of a third exemplary embodiment of a powder as disclosed herein having a multi-modal distribution of particle sizes;

FIG. 8 is a flow chart of an exemplary embodiment of a method of making a powder as disclosed herein;

FIG. 9 is a photomicrograph of an exemplary embodiment of a powder compact as disclosed herein;

FIG. 10 is a schematic of illustration of an exemplary embodiment of the powder compact of FIG. 9 made using a powder having single-layer coated powder particles as it would appear taken along section 10-10;

FIG. 11 is a schematic illustration of an exemplary embodiment of a powder compact as disclosed herein having a homogenous multi-modal distribution of particle sizes;

FIG. 12 is a schematic illustration of an exemplary embodiment of a powder compact as disclosed herein having a non-homogeneous, multi-modal distribution of particle sizes;

FIG. 13 is a schematic illustration of an exemplary embodiment of a powder compact as disclosed herein formed from a first powder and a second powder and having a homogenous multi-modal distribution of particle sizes;

FIG. 14 is a schematic illustration of an exemplary embodiment of a powder compact as disclosed herein formed from a first powder and a second powder and having a non-homogeneous multi-modal distribution of particle sizes.

FIG. 15 is a schematic of illustration of another exemplary embodiment of the powder compact of FIG. 9 made using a powder having multilayer coated powder particles as it would appear taken along section 10-10;

FIG. 16 is a schematic cross-sectional illustration of an exemplary embodiment of a precursor powder compact;

FIG. 17 is a flow chart of an exemplary embodiment of a method of making a powder compact as disclosed herein;

FIG. 18 is a table that describes the particle core and metallic coating layer configurations for powder particles and powders used to make exemplary embodiments of powder compacts for testing as disclosed herein;

FIG. 19 a plot of the compressive strength of the powder compacts of FIG. 18 both dry and in an aqueous solution comprising 3% KCl;

FIG. 20 is a plot of the rate of corrosion (ROC) of the powder compacts of FIG. 18 in an aqueous solution comprising 3% KCl at 200° F. and room temperature;

FIG. 21 is a plot of the ROC of the powder compacts of FIG. 18 in 15% HCl;

FIG. 22 is a schematic illustration of a change in a property of a powder compact as disclosed herein as a function of time and a change in condition of the powder compact environment;

FIG. 23 is an electron photomicrograph of a fracture surface of a powder compact formed from a pure Mg powder;

FIG. 24 is an electron photomicrograph of a fracture surface of an exemplary embodiment of a powder metal compact as described herein; and

FIG. 25 is a plot of compressive strength of a powder compact as a function the amount of a constituent (Al<sub>2</sub>O<sub>3</sub>) of the cellular nanomatrix.

## DETAILED DESCRIPTION

10 Lightweight, high-strength metallic materials are disclosed that may be used in a wide variety of applications and application environments, including use in various wellbore environments to make various selectively and controllably disposable or degradable lightweight, high-strength down-hole tools or other downhole components, as well as many other applications for use in both durable and disposable or degradable articles. These lightweight, high-strength and selectively and controllably degradable materials include fully-dense, sintered powder compacts formed from coated powder materials that include various lightweight particle cores and core materials having various single layer and multilayer nanoscale coatings. These powder compacts are made from coated metallic powders that include various electrochemically-active (e.g., having relatively higher standard oxidation potentials) lightweight, high-strength particle cores and core materials, such as electrochemically active metals, that are dispersed within a cellular nanomatrix formed from the various nanoscale metallic coating layers of metallic coating materials, and are particularly useful in wellbore applications. These powder compacts provide a unique and advantageous combination of mechanical strength properties, such as compression and shear strength, low density and selectable and controllable corrosion properties, particularly rapid and controlled dissolution in various wellbore fluids. For example, the particle core and coating layers of these powders may be selected to provide sintered powder compacts suitable for use as high strength engineered materials having a compressive strength and shear strength comparable to various other engineered materials, including carbon, stainless and alloy steels, but which also have a low density comparable to various polymers, elastomers, low-density porous ceramics and composite materials. As yet another example, these powders and powder compact materials may be configured to provide a selectable and controllable degradation or disposal in response to a change in an environmental condition, such as a transition from a very low dissolution rate to a very rapid dissolution rate in response to a change in a property or condition of a wellbore proximate an article formed from the compact, including a property change in a wellbore fluid that is in contact with the powder compact. The selectable and controllable degradation or disposal characteristics described also allow the dimensional stability and strength of articles, such as wellbore tools or other components, 30 made from these materials to be maintained until they are no longer needed, at which time a predetermined environmental condition, such as a wellbore condition, including wellbore fluid temperature, pressure or pH value, may be changed to promote their removal by rapid dissolution. These coated powder materials and powder compacts and engineered materials formed from them, as well as methods of making them, are described further below.

Referring to FIGS. 1-5, a metallic powder 10 includes a plurality of metallic, coated powder particles 12. Powder particles 12 may be formed to provide a powder 10, including free-flowing powder, that may be poured or otherwise disposed in all manner of forms or molds (not shown) having

all manner of shapes and sizes and that may be used to fashion precursor powder compacts **100** (FIG. 16) and powder compacts **200** (FIGS. 10-15), as described herein, that may be used as, or for use in manufacturing, various articles of manufacture, including various wellbore tools and components.

Each of the metallic, coated powder particles **12** of powder **10** includes a particle core **14** and a metallic coating layer **16** disposed on the particle core **14**. The particle core **14** includes a core material **18**. The core material **18** may include any suitable material for forming the particle core **14** that provides powder particle **12** that can be sintered to form a lightweight, high-strength powder compact **200** having selectable and controllable dissolution characteristics. Suitable core materials include electrochemically active metals having a standard oxidation potential greater than or equal to that of Zn, including as Mg, Al, Mn or Zn or a combination thereof. These electrochemically active metals are very reactive with a number of common wellbore fluids, including any number of ionic fluids or highly polar fluids, such as those that contain various chlorides. Examples include fluids comprising potassium chloride (KCl), hydrochloric acid (HCl), calcium chloride (CaCl<sub>2</sub>), calcium bromide (CaBr<sub>2</sub>) or zinc bromide (ZnBr<sub>2</sub>). Core material **18** may also include other metals that are less electrochemically active than Zn or non-metallic materials, or a combination thereof. Suitable non-metallic materials include ceramics, composites, glasses or carbon, or a combination thereof. Core material **18** may be selected to provide a high dissolution rate in a predetermined wellbore fluid, but may also be selected to provide a relatively low dissolution rate, including zero dissolution, where dissolution of the nanomatrix material causes the particle core **14** to be rapidly undermined and liberated from the particle compact at the interface with the wellbore fluid, such that the effective rate of dissolution of particle compacts made using particle cores **14** of these core materials **18** is high, even though core material **18** itself may have a low dissolution rate, including core materials **20** that may be substantially insoluble in the wellbore fluid.

With regard to the electrochemically active metals as core materials **18**, including Mg, Al, Mn or Zn, these metals may be used as pure metals or in any combination with one another, including various alloy combinations of these materials, including binary, tertiary, or quaternary alloys of these materials. These combinations may also include composites of these materials. Further, in addition to combinations with one another, the Mg, Al, Mn or Zn core materials **18** may also include other constituents, including various alloying additions, to alter one or more properties of the particle cores **14**, such as by improving the strength, lowering the density or altering the dissolution characteristics of the core material **18**.

Among the electrochemically active metals, Mg, either as a pure metal or an alloy or a composite material, is particularly useful, because of its low density and ability to form high-strength alloys, as well as its high degree of electrochemical activity, since it has a standard oxidation potential higher than Al, Mn or Zn. Mg alloys include all alloys that have Mg as an alloy constituent. Mg alloys that combine other electrochemically active metals, as described herein, as alloy constituents are particularly useful, including binary Mg—Zn, Mg—Al and Mg—Mn alloys, as well as tertiary Mg—Zn—Y and Mg—Al—X alloys, where X includes Zn, Mn, Si, Ca or Y, or a combination thereof. These Mg—Al—X alloys may include, by weight, up to about 85% Mg, up to about 15% Al and up to about 5% X. Particle core **14** and core material **18**, and particularly electrochemically

active metals including Mg, Al, Mn or Zn, or combinations thereof, may also include a rare earth element or combination of rare earth elements. As used herein, rare earth elements include Sc, Y, La, Ce, Pr, Nd or Er, or a combination of rare earth elements. Where present, a rare earth element or combinations of rare earth elements may be present, by weight, in an amount of about 5% or less.

Particle core **14** and core material **18** have a melting temperature (T<sub>P</sub>). As used herein, T<sub>P</sub> includes the lowest temperature at which incipient melting or liquation or other forms of partial melting occur within core material **18**, regardless of whether core material **18** comprises a pure metal, an alloy with multiple phases having different melting temperatures or a composite of materials having different melting temperatures.

Particle cores **14** may have any suitable particle size or range of particle sizes or distribution of particle sizes. For example, the particle cores **14** may be selected to provide an average particle size that is represented by a normal or Gaussian type unimodal distribution around an average or mean, as illustrated generally in FIG. 1. In another example, particle cores **14** may be selected or mixed to provide a multimodal distribution of particle sizes, including a plurality of average particle core sizes, such as, for example, a homogeneous bimodal distribution of average particle sizes, as illustrated generally and schematically in FIG. 6. The selection of the distribution of particle core size may be used to determine, for example, the particle size and interparticle spacing **15** of the particles **12** of powder **10**. In an exemplary embodiment, the particle cores **14** may have a unimodal distribution and an average particle diameter of about 5  $\mu\text{m}$  to about 300  $\mu\text{m}$ , more particularly about 80  $\mu\text{m}$  to about 120  $\mu\text{m}$ , and even more particularly about 100  $\mu\text{m}$ .

Particle cores **14** may have any suitable particle shape, including any regular or irregular geometric shape, or combination thereof. In an exemplary embodiment, particle cores **14** are substantially spheroidal electrochemically active metal particles. In another exemplary embodiment, particle cores **14** are substantially irregularly shaped ceramic particles. In yet another exemplary embodiment, particle cores **14** are carbon or other nanotube structures or hollow glass microspheres.

Each of the metallic, coated powder particles **12** of powder **10** also includes a metallic coating layer **16** that is disposed on particle core **14**. Metallic coating layer **16** includes a metallic coating material **20**. Metallic coating material **20** gives the powder particles **12** and powder **10** its metallic nature. Metallic coating layer **16** is a nanoscale coating layer. In an exemplary embodiment, metallic coating layer **16** may have a thickness of about 25 nm to about 2500 nm. The thickness of metallic coating layer **16** may vary over the surface of particle core **14**, but will preferably have a substantially uniform thickness over the surface of particle core **14**. Metallic coating layer **16** may include a single layer, as illustrated in FIG. 2, or a plurality of layers as a multilayer coating structure, as illustrated in FIGS. 3-5 for up to four layers. In a single layer coating, or in each of the layers of a multilayer coating, the metallic coating layer **16** may include a single constituent chemical element or compound, or may include a plurality of chemical elements or compounds. Where a layer includes a plurality of chemical constituents or compounds, they may have all manner of homogeneous or heterogeneous distributions, including a homogeneous or heterogeneous distribution of metallurgical phases. This may include a graded distribution where the relative amounts of the chemical constituents or compounds vary according to respective constituent profiles across the

thickness of the layer. In both single layer and multilayer coatings **16**, each of the respective layers, or combinations of them, may be used to provide a predetermined property to the powder particle **12** or a sintered powder compact formed therefrom. For example, the predetermined property may include the bond strength of the metallurgical bond between the particle core **14** and the coating material **20**; the interdiffusion characteristics between the particle core **14** and metallic coating layer **16**, including any interdiffusion between the layers of a multilayer coating layer **16**; the interdiffusion characteristics between the various layers of a multilayer coating layer **16**; the interdiffusion characteristics between the metallic coating layer **16** of one powder particle and that of an adjacent powder particle **12**; the bond strength of the metallurgical bond between the metallic coating layers of adjacent sintered powder particles **12**, including the outermost layers of multilayer coating layers; and the electrochemical activity of the coating layer **16**.

Metallic coating layer **16** and coating material **20** have a melting temperature ( $T_C$ ). As used herein,  $T_C$  includes the lowest temperature at which incipient melting or liquation or other forms of partial melting occur within coating material **20**, regardless of whether coating material **20** comprises a pure metal, an alloy with multiple phases each having different melting temperatures or a composite, including a composite comprising a plurality of coating material layers having different melting temperatures.

Metallic coating material **20** may include any suitable metallic coating material **20** that provides a sinterable outer surface **21** that is configured to be sintered to an adjacent powder particle **12** that also has a metallic coating layer **16** and sinterable outer surface **21**. In powders **10** that also include second or additional (coated or uncoated) particles **32**, as described herein, the sinterable outer surface **21** of metallic coating layer **16** is also configured to be sintered to a sinterable outer surface **21** of second particles **32**. In an exemplary embodiment, the powder particles **12** are sinterable at a predetermined sintering temperature ( $T_S$ ) that is a function of the core material **18** and coating material **20**, such that sintering of powder compact **200** is accomplished entirely in the solid state and where  $T_S$  is less than  $T_P$  and  $T_C$ . Sintering in the solid state limits particle core **14**/metallic coating layer **16** interactions to solid state diffusion processes and metallurgical transport phenomena and limits growth of and provides control over the resultant interface between them. In contrast, for example, the introduction of liquid phase sintering would provide for rapid interdiffusion of the particle core **14**/metallic coating layer **16** materials and make it difficult to limit the growth of and provide control over the resultant interface between them, and thus interfere with the formation of the desirable microstructure of particle compact **200** as described herein.

In an exemplary embodiment, core material **18** will be selected to provide a core chemical composition and the coating material **20** will be selected to provide a coating chemical composition and these chemical compositions will also be selected to differ from one another. In another exemplary embodiment, the core material **18** will be selected to provide a core chemical composition and the coating material **20** will be selected to provide a coating chemical composition and these chemical compositions will also be selected to differ from one another at their interface. Differences in the chemical compositions of coating material **20** and core material **18** may be selected to provide different dissolution rates and selectable and controllable dissolution of powder compacts **200** that incorporate them making them selectively and controllably dissolvable. This includes dis-

solution rates that differ in response to a changed condition in the wellbore, including an indirect or direct change in a wellbore fluid. In an exemplary embodiment, a powder compact **200** formed from powder **10** having chemical compositions of core material **18** and coating material **20** that make compact **200** is selectively dissolvable in a wellbore fluid in response to a changed wellbore condition that includes a change in temperature, change in pressure, change in flow rate, change in pH or change in chemical composition of the wellbore fluid, or a combination thereof. The selectable dissolution response to the changed condition may result from actual chemical reactions or processes that promote different rates of dissolution, but also encompass changes in the dissolution response that are associated with physical reactions or processes, such as changes in wellbore fluid pressure or flow rate.

In an exemplary embodiment of a powder **10**, particle core **14** includes Mg, Al, Mn or Zn, or a combination thereof, as core material **18**, and more particularly may include pure Mg and Mg alloys, and metallic coating layer **16** includes Al, Zn, Mn, Mg, Mo, W, Cu, Fe, Si, Ca, Co, Ta, Re, or Ni, or an oxide, nitride or a carbide thereof, or a combination of any of the aforementioned materials as coating material **20**.

In another exemplary embodiment of powder **10**, particle core **14** includes Mg, Al, Mn or Zn, or a combination thereof, as core material **18**, and more particularly may include pure Mg and Mg alloys, and metallic coating layer **16** includes a single layer of Al or Ni, or a combination thereof, as coating material **20**, as illustrated in FIG. 2. Where metallic coating layer **16** includes a combination of two or more constituents, such as Al and Ni, the combination may include various graded or co-deposited structures of these materials where the amount of each constituent, and hence the composition of the layer, varies across the thickness of the layer, as also illustrated in FIG. 2.

In yet another exemplary embodiment, particle core **14** includes Mg, Al, Mn or Zn, or a combination thereof, as core material **18**, and more particularly may include pure Mg and Mg alloys, and coating layer **16** includes two layers as core material **20**, as illustrated in FIG. 3. The first layer **22** is disposed on the surface of particle core **14** and includes Al or Ni, or a combination thereof, as described herein. The second layer **24** is disposed on the surface of the first layer **22** and includes Al, Zn, Mg, Mo, W, Cu, Fe, Si, Ca, Co, Ta, Re or Ni, or a combination thereof, and the first layer has a chemical composition that is different than the chemical composition of the second layer. In general, first layer **22** will be selected to provide a strong metallurgical bond to particle core **14** and to limit interdiffusion between the particle core **14** and coating layer **16**, particularly first layer **22**. Second layer **24** may be selected to increase the strength of the metallic coating layer **16**, or to provide a strong metallurgical bond and promote sintering with the second layer **24** of adjacent powder particles **12**, or both. In an exemplary embodiment, the respective layers of metallic coating layer **16** may be selected to promote the selective and controllable dissolution of the coating layer **16** in response to a change in a property of the wellbore, including the wellbore fluid, as described herein. However, this is only exemplary and it will be appreciated that other selection criteria for the various layers may also be employed. For example, any of the respective layers may be selected to promote the selective and controllable dissolution of the coating layer **16** in response to a change in a property of the wellbore, including the wellbore fluid, as described herein. Exemplary embodiments of a two-layer metallic coating

layers **16** for use on particles cores **14** comprising Mg include first/second layer combinations comprising Al/Ni and Al/W.

In still another embodiment, particle core **14** includes Mg, Al, Mn or Zn, or a combination thereof, as core material **18**, and more particularly may include pure Mg and Mg alloys, and coating layer **16** includes three layers, as illustrated in FIG. 4. The first layer **22** is disposed on particle core **14** and may include Al or Ni, or a combination thereof. The second layer **24** is disposed on first layer **22** and may include Al, Zn, Mg, Mo, W, Cu, Fe, Si, Ca, Co, Ta, Re or Ni, or an oxide, nitride or a carbide thereof, or a combination of any of the aforementioned second layer materials. The third layer **26** is disposed on the second layer **24** and may include Al, Mn, Fe, Co, Ni or a combination thereof. In a three-layer configuration, the composition of adjacent layers is different, such that the first layer has a chemical composition that is different than the second layer, and the second layer has a chemical composition that is different than the third layer. In an exemplary embodiment, first layer **22** may be selected to provide a strong metallurgical bond to particle core **14** and to limit interdiffusion between the particle core **14** and coating layer **16**, particularly first layer **22**. Second layer **24** may be selected to increase the strength of the metallic coating layer **16**, or to limit interdiffusion between particle core **14** or first layer **22** and outer or third layer **26**, or to promote adhesion and a strong metallurgical bond between third layer **26** and first layer **22**, or any combination of them. Third layer **26** may be selected to provide a strong metallurgical bond and promote sintering with the third layer **26** of adjacent powder particles **12**. However, this is only exemplary and it will be appreciated that other selection criteria for the various layers may also be employed. For example, any of the respective layers may be selected to promote the selective and controllable dissolution of the coating layer **16** in response to a change in a property of the wellbore, including the wellbore fluid, as described herein. An exemplary embodiment of a three-layer coating layer for use on particles cores comprising Mg include first/second/third layer combinations comprising Al/Al<sub>2</sub>O<sub>3</sub>/Al.

In still another embodiment, particle core **14** includes Mg, Al, Mn or Zn, or a combination thereof, as core material **18**, and more particularly may include pure Mg and Mg alloys, and coating layer **16** includes four layers, as illustrated in FIG. 5. In the four layer configuration, the first layer **22** may include Al or Ni, or a combination thereof, as described herein. The second layer **24** may include Al, Zn, Mg, Mo, W, Cu, Fe, Si, Ca, Co, Ta, Re or Ni or an oxide, nitride, carbide thereof, or a combination of the aforementioned second layer materials. The third layer **26** may also include Al, Zn, Mg, Mo, W, Cu, Fe, Si, Ca, Co, Ta, Re or Ni, or an oxide, nitride or carbide thereof, or a combination of any of the aforementioned third layer materials. The fourth layer **28** may include Al, Mn, Fe, Co, Ni or a combination thereof. In the four layer configuration, the chemical composition of adjacent layers is different, such that the chemical composition of first layer **22** is different than the chemical composition of second layer **24**, the chemical composition of second layer **24** different than the chemical composition of third layer **26**, and the chemical composition of third layer **26** is different than the chemical composition of fourth layer **28**. In an exemplary embodiment, the selection of the various layers will be similar to that described for the three-layer configuration above with regard to the inner (first) and outer (fourth) layers, with the second and third layers available for providing enhanced interlayer adhesion, strength of the overall metallic coating layer **16**, limited

interlayer diffusion or selectable and controllable dissolution, or a combination thereof. However, this is only exemplary and it will be appreciated that other selection criteria for the various layers may also be employed. For example, any of the respective layers may be selected to promote the selective and controllable dissolution of the coating layer **16** in response to a change in a property of the wellbore, including the wellbore fluid, as described herein.

The thickness of the various layers in multi-layer configurations may be apportioned between the various layers in any manner so long as the sum of the layer thicknesses provide a nanoscale coating layer **16**, including layer thicknesses as described herein. In one embodiment, the first layer **22** and outer layer (**24**, **26**, or **28** depending on the number of layers) may be thicker than other layers, where present, due to the desire to provide sufficient material to promote the desired bonding of first layer **22** with the particle core **14**, or the bonding of the outer layers of adjacent powder particles **12**, during sintering of powder compact **200**.

Powder **10** may also include an additional or second powder **30** interspersed in the plurality of powder particles **12**, as illustrated in FIG. 7. In an exemplary embodiment, the second powder **30** includes a plurality of second powder particles **32**. These second powder particles **32** may be selected to change a physical, chemical, mechanical or other property of a powder particle compact **200** formed from powder **10** and second powder **30**, or a combination of such properties. In an exemplary embodiment, the property change may include an increase in the compressive strength of powder compact **200** formed from powder **10** and second powder **30**. In another exemplary embodiment, the second powder **30** may be selected to promote the selective and controllable dissolution of in particle compact **200** formed from powder **10** and second powder **30** in response to a change in a property of the wellbore, including the wellbore fluid, as described herein. Second powder particles **32** may be uncoated or coated with a metallic coating layer **36**. When coated, including single layer or multilayer coatings, the coating layer **36** of second powder particles **32** may comprise the same coating material **40** as coating material **20** of powder particles **12**, or the coating material **40** may be different. The second powder particles **32** (uncoated) or particle cores **34** may include any suitable material to provide the desired benefit, including many metals. In an exemplary embodiment, when coated powder particles **12** comprising Mg, Al, Mn or Zn, or a combination thereof are employed, suitable second powder particles **32** may include Ni, W, Cu, Co or Fe, or a combination thereof. Since second powder particles **32** will also be configured for solid state sintering to powder particles **12** at the predetermined sintering temperature ( $T_S$ ), particle cores **34** will have a melting temperature  $T_{AP}$  and any coating layers **36** will have a second melting temperature  $T_{AC}$  where  $T_S$  is less than  $T_{AP}$  and  $T_{AC}$ . It will also be appreciated that second powder **30** is not limited to one additional powder particle **32** type (i.e., a second powder particle), but may include a plurality of additional powder particles **32** (i.e., second, third, fourth, etc. types of additional powder particles **32**) in any number.

Referring to FIG. 8, an exemplary embodiment of a method **300** of making a metallic powder **10** is disclosed. Method **300** includes forming **310** a plurality of particle cores **14** as described herein. Method **300** also includes depositing **320** a metallic coating layer **16** on each of the plurality of particle cores **14**. Depositing **320** is the process by which coating layer **16** is disposed on particle core **14** as described herein.

Forming 310 of particle cores 14 may be performed by any suitable method for forming a plurality of particle cores 14 of the desired core material 18, which essentially comprise methods of forming a powder of core material 18. Suitable powder forming methods include mechanical methods; including machining, milling, impacting and other mechanical methods for forming the metal powder; chemical methods, including chemical decomposition, precipitation from a liquid or gas, solid-solid reactive synthesis and other chemical powder forming methods; atomization methods, including gas atomization, liquid and water atomization, centrifugal atomization, plasma atomization and other atomization methods for forming a powder; and various evaporation and condensation methods. In an exemplary embodiment, particle cores 14 comprising Mg may be fabricated using an atomization method, such as vacuum spray forming or inert gas spray forming.

Depositing 320 of metallic coating layers 16 on the plurality of particle cores 14 may be performed using any suitable deposition method, including various thin film deposition methods, such as, for example, chemical vapor deposition and physical vapor deposition methods. In an exemplary embodiment, depositing 320 of metallic coating layers 16 is performed using fluidized bed chemical vapor deposition (FBCVD). Depositing 320 of the metallic coating layers 16 by FBCVD includes flowing a reactive fluid as a coating medium that includes the desired metallic coating material 20 through a bed of particle cores 14 fluidized in a reactor vessel under suitable conditions, including temperature, pressure and flow rate conditions and the like, sufficient to induce a chemical reaction of the coating medium to produce the desired metallic coating material 20 and induce its deposition upon the surface of particle cores 14 to form coated powder particles 12. The reactive fluid selected will depend upon the metallic coating material 20 desired, and will typically comprise an organometallic compound that includes the metallic material to be deposited, such as nickel tetracarbonyl ( $\text{Ni}(\text{CO})_4$ ), tungsten hexafluoride ( $\text{WF}_6$ ), and triethyl aluminum ( $\text{C}_6\text{H}_{15}\text{Al}$ ), that is transported in a carrier fluid, such as helium or argon gas. The reactive fluid, including carrier fluid, causes at least a portion of the plurality of particle cores 14 to be suspended in the fluid, thereby enabling the entire surface of the suspended particle cores 14 to be exposed to the reactive fluid, including, for example, a desired organometallic constituent, and enabling deposition of metallic coating material 20 and coating layer 16 over the entire surfaces of particle cores 14 such that they each become enclosed forming coated particles 12 having metallic coating layers 16, as described herein. As also described herein, each metallic coating layer 16 may include a plurality of coating layers. Coating material 20 may be deposited in multiple layers to form a multilayer metallic coating layer 16 by repeating the step of depositing 320 described above and changing 330 the reactive fluid to provide the desired metallic coating material 20 for each subsequent layer, where each subsequent layer is deposited on the outer surface of particle cores 14 that already include any previously deposited coating layer or layers that make up metallic coating layer 16. The metallic coating materials 20 of the respective layers (e.g., 22, 24, 26, 28, etc.) may be different from one another, and the differences may be provided by utilization of different reactive media that are configured to produce the desired metallic coating layers 16 on the particle cores 14 in the fluidized bed reactor.

As illustrated in FIGS. 1 and 9, particle core 14 and core material 18 and metallic coating layer 16 and coating material 20 may be selected to provide powder particles 12

and a powder 10 that is configured for compaction and sintering to provide a powder compact 200 that is lightweight (i.e., having a relatively low density), high-strength and is selectively and controllably removable from a wellbore in response to a change in a wellbore property, including being selectively and controllably dissolvable in an appropriate wellbore fluid, including various wellbore fluids as disclosed herein. Powder compact 200 includes a substantially-continuous, cellular nanomatrix 216 of a nanomatrix material 220 having a plurality of dispersed particles 214 dispersed throughout the cellular nanomatrix 216. The substantially-continuous cellular nanomatrix 216 and nanomatrix material 220 formed of sintered metallic coating layers 16 is formed by the compaction and sintering of the plurality of metallic coating layers 16 of the plurality of powder particles 12. The chemical composition of nanomatrix material 220 may be different than that of coating material 20 due to diffusion effects associated with the sintering as described herein. Powder metal compact 200 also includes a plurality of dispersed particles 214 that comprise particle core material 218. Dispersed particle cores 214 and core material 218 correspond to and are formed from the plurality of particle cores 14 and core material 18 of the plurality of powder particles 12 as the metallic coating layers 16 are sintered together to form nanomatrix 216. The chemical composition of core material 218 may be different than that of core material 18 due to diffusion effects associated with sintering as described herein.

As used herein, the use of the term substantially-continuous cellular nanomatrix 216 does not connote the major constituent of the powder compact, but rather refers to the minority constituent or constituents, whether by weight or by volume. This is distinguished from most matrix composite materials where the matrix comprises the majority constituent by weight or volume. The use of the term substantially-continuous, cellular nanomatrix is intended to describe the extensive, regular, continuous and interconnected nature of the distribution of nanomatrix material 220 within powder compact 200. As used herein, "substantially-continuous" describes the extension of the nanomatrix material throughout powder compact 200 such that it extends between and envelopes substantially all of the dispersed particles 214. Substantially-continuous is used to indicate that complete continuity and regular order of the nanomatrix around each dispersed particle 214 is not required. For example, defects in the coating layer 16 over particle core 14 on some powder particles 12 may cause bridging of the particle cores 14 during sintering of the powder compact 200, thereby causing localized discontinuities to result within the cellular nanomatrix 216, even though in the other portions of the powder compact the nanomatrix is substantially continuous and exhibits the structure described herein. As used herein, "cellular" is used to indicate that the nanomatrix defines a network of generally repeating, interconnected, compartments or cells of nanomatrix material 220 that encompass and also interconnect the dispersed particles 214. As used herein, "nanomatrix" is used to describe the size or scale of the matrix, particularly the thickness of the matrix between adjacent dispersed particles 214. The metallic coating layers 16 that are sintered together to form the nanomatrix are themselves nanoscale thickness coating layers. Since the nanomatrix at most locations, other than the intersection of more than two dispersed particles 214, generally comprises the interdiffusion and bonding of two coating layers 16 from adjacent powder particles 12 having nanoscale thicknesses, the matrix formed also has a nanoscale thickness (e.g., approximately two times the coating layer thickness as

described herein) and is thus described as a nanomatrix. Further, the use of the term dispersed particles 214 does not connote the minor constituent of powder compact 200, but rather refers to the majority constituent or constituents, whether by weight or by volume. The use of the term dispersed particle is intended to convey the discontinuous and discrete distribution of particle core material 218 within powder compact 200.

Powder compact 200 may have any desired shape or size, including that of a cylindrical billet or bar that may be machined or otherwise used to form useful articles of manufacture, including various wellbore tools and components. The pressing used to form precursor powder compact 100 and sintering and pressing processes used to form powder compact 200 and deform the powder particles 12, including particle cores 14 and coating layers 16, to provide the full density and desired macroscopic shape and size of powder compact 200 as well as its microstructure. The microstructure of powder compact 200 includes an equiaxed configuration of dispersed particles 214 that are dispersed throughout and embedded within the substantially-continuous, cellular nanomatrix 216 of sintered coating layers. This microstructure is somewhat analogous to an equiaxed grain microstructure with a continuous grain boundary phase, except that it does not require the use of alloy constituents having thermodynamic phase equilibria properties that are capable of producing such a structure. Rather, this equiaxed dispersed particle structure and cellular nanomatrix 216 of sintered metallic coating layers 16 may be produced using constituents where thermodynamic phase equilibrium conditions would not produce an equiaxed structure. The equiaxed morphology of the dispersed particles 214 and cellular network 216 of particle layers results from sintering and deformation of the powder particles 12 as they are compacted and interdiffuse and deform to fill the interparticle spaces 15 (FIG. 1). The sintering temperatures and pressures may be selected to ensure that the density of powder compact 200 achieves substantially full theoretical density.

In an exemplary embodiment as illustrated in FIGS. 1 and 9, dispersed particles 214 are formed from particle cores 14 dispersed in the cellular nanomatrix 216 of sintered metallic coating layers 16, and the nanomatrix 216 includes a solid-state metallurgical bond 217 or bond layer 219, as illustrated schematically in FIG. 10, extending between the dispersed particles 214 throughout the cellular nanomatrix 216 that is formed at a sintering temperature ( $T_S$ ), where  $T_S$  is less than  $T_C$  and  $T_P$ . As indicated, solid-state metallurgical bond 217 is formed in the solid state by solid-state interdiffusion between the coating layers 16 of adjacent powder particles 12 that are compressed into touching contact during the compaction and sintering processes used to form powder compact 200, as described herein. As such, sintered coating layers 16 of cellular nanomatrix 216 include a solid-state bond layer 219 that has a thickness ( $t$ ) defined by the extent of the interdiffusion of the coating materials 20 of the coating layers 16, which will in turn be defined by the nature of the coating layers 16, including whether they are single or multilayer coating layers, whether they have been selected to promote or limit such interdiffusion, and other factors, as described herein, as well as the sintering and compaction conditions, including the sintering time, temperature and pressure used to form powder compact 200.

As nanomatrix 216 is formed, including bond 217 and bond layer 219, the chemical composition or phase distribution, or both, of metallic coating layers 16 may change. Nanomatrix 216 also has a melting temperature ( $T_M$ ). As used herein,  $T_M$  includes the lowest temperature at which

incipient melting or liquation or other forms of partial melting will occur within nanomatrix 216, regardless of whether nanomatrix material 220 comprises a pure metal, an alloy with multiple phases each having different melting temperatures or a composite, including a composite comprising a plurality of layers of various coating materials having different melting temperatures, or a combination thereof, or otherwise. As dispersed particles 214 and particle core materials 218 are formed in conjunction with nanomatrix 216, diffusion of constituents of metallic coating layers 16 into the particle cores 14 is also possible, which may result in changes in the chemical composition or phase distribution, or both, of particle cores 14. As a result, dispersed particles 214 and particle core materials 218 may have a melting temperature ( $T_{DP}$ ) that is different than  $T_P$ . As used herein,  $T_{DP}$  includes the lowest temperature at which incipient melting or liquation or other forms of partial melting will occur within dispersed particles 214, regardless of whether particle core material 218 comprise a pure metal, an alloy with multiple phases each having different melting temperatures or a composite, or otherwise. Powder compact 200 is formed at a sintering temperature ( $T_S$ ), where  $T_S$  is less than  $T_C$ ,  $T_P$ ,  $T_M$  and  $T_{DP}$ .

Dispersed particles 214 may comprise any of the materials described herein for particle cores 14, even though the chemical composition of dispersed particles 214 may be different due to diffusion effects as described herein. In an exemplary embodiment, dispersed particles 214 are formed from particle cores 14 comprising materials having a standard oxidation potential greater than or equal to Zn, including Mg, Al, Zn or Mn, or a combination thereof, may include various binary, tertiary and quaternary alloys or other combinations of these constituents as disclosed herein in conjunction with particle cores 14. Of these materials, those having dispersed particles 214 comprising Mg and the nanomatrix 216 formed from the metallic coating materials 16 described herein are particularly useful. Dispersed particles 214 and particle core material 218 of Mg, Al, Zn or Mn, or a combination thereof, may also include a rare earth element, or a combination of rare earth elements as disclosed herein in conjunction with particle cores 14.

In another exemplary embodiment, dispersed particles 214 are formed from particle cores 14 comprising metals that are less electrochemically active than Zn or non-metallic materials. Suitable non-metallic materials include ceramics, glasses (e.g., hollow glass microspheres) or carbon, or a combination thereof, as described herein.

Dispersed particles 214 of powder compact 200 may have any suitable particle size, including the average particle sizes described herein for particle cores 14.

Dispersed particles 214 may have any suitable shape depending on the shape selected for particle cores 14 and powder particles 12, as well as the method used to sinter and compact powder 10. In an exemplary embodiment, powder particles 12 may be spheroidal or substantially spheroidal and dispersed particles 214 may include an equiaxed particle configuration as described herein.

The nature of the dispersion of dispersed particles 214 may be affected by the selection of the powder 10 or powders 10 used to make particle compact 200. In one exemplary embodiment, a powder 10 having a unimodal distribution of powder particle 12 sizes may be selected to form powder compact 200 and will produce a substantially homogeneous unimodal dispersion of particle sizes of dispersed particles 214 within cellular nanomatrix 216, as illustrated generally in FIG. 9. In another exemplary embodiment, a plurality of powders 10 having a plurality of

powder particles with particle cores **14** that have the same core materials **18** and different core sizes and the same coating material **20** may be selected and uniformly mixed as described herein to provide a powder **10** having a homogenous, multimodal distribution of powder particle **12** sizes, and may be used to form powder compact **200** having a homogeneous, multimodal dispersion of particle sizes of dispersed particles **214** within cellular nanomatrix **216**, as illustrated schematically in FIGS. 6 and 11. Similarly, in yet another exemplary embodiment, a plurality of powders **10** having a plurality of particle cores **14** that may have the same core materials **18** and different core sizes and the same coating material **20** may be selected and distributed in a non-uniform manner to provide a non-homogenous, multimodal distribution of powder particle sizes, and may be used to form powder compact **200** having a non-homogeneous, multimodal dispersion of particle sizes of dispersed particles **214** within cellular nanomatrix **216**, as illustrated schematically in FIG. 12. The selection of the distribution of particle core size may be used to determine, for example, the particle size and interparticle spacing of the dispersed particles **214** within the cellular nanomatrix **216** of powder compacts **200** made from powder **10**.

As illustrated generally in FIGS. 7 and 13, powder metal compact **200** may also be formed using coated metallic powder **10** and an additional or second powder **30**, as described herein. The use of an additional powder **30** provides a powder compact **200** that also includes a plurality of dispersed second particles **234**, as described herein, that are dispersed within the nanomatrix **216** and are also dispersed with respect to the dispersed particles **214**. Dispersed second particles **234** may be formed from coated or uncoated second powder particles **32**, as described herein. In an exemplary embodiment, coated second powder particles **32** may be coated with a coating layer **36** that is the same as coating layer **16** of powder particles **12**, such that coating layers **36** also contribute to the nanomatrix **216**. In another exemplary embodiment, the second powder particles **232** may be uncoated such that dispersed second particles **234** are embedded within nanomatrix **216**. As disclosed herein, powder **10** and additional powder **30** may be mixed to form a homogeneous dispersion of dispersed particles **214** and dispersed second particles **234**, as illustrated in FIG. 13, or to form a non-homogeneous dispersion of these particles, as illustrated in FIG. 14. The dispersed second particles **234** may be formed from any suitable additional powder **30** that is different from powder **10**, either due to a compositional difference in the particle core **34**, or coating layer **36**, or both of them, and may include any of the materials disclosed herein for use as second powder **30** that are different from the powder **10** that is selected to form powder compact **200**. In an exemplary embodiment, dispersed second particles **234** may include Fe, Ni, Co or Cu, or oxides, nitrides or carbides thereof, or a combination of any of the aforementioned materials.

Nanomatrix **216** is a substantially-continuous, cellular network of metallic coating layers **16** that are sintered to one another. The thickness of nanomatrix **216** will depend on the nature of the powder **10** or powders **10** used to form powder compact **200**, as well as the incorporation of any second powder **30**, particularly the thicknesses of the coating layers associated with these particles. In an exemplary embodiment, the thickness of nanomatrix **216** is substantially uniform throughout the microstructure of powder compact **200** and comprises about two times the thickness of the coating layers **16** of powder particles **12**. In another exemplary embodiment, the cellular network **216** has a substantially

uniform average thickness between dispersed particles **214** of about 50 nm to about 5000 nm.

Nanomatrix **216** is formed by sintering metallic coating layers **16** of adjacent particles to one another by interdiffusion and creation of bond layer **219** as described herein. Metallic coating layers **16** may be single layer or multilayer structures, and they may be selected to promote or inhibit diffusion, or both, within the layer or between the layers of metallic coating layer **16**, or between the metallic coating layer **16** and particle core **14**, or between the metallic coating layer **16** and the metallic coating layer **16** of an adjacent powder particle, the extent of interdiffusion of metallic coating layers **16** during sintering may be limited or extensive depending on the coating thicknesses, coating material or materials selected, the sintering conditions and other factors. Given the potential complexity of the interdiffusion and interaction of the constituents, description of the resulting chemical composition of nanomatrix **216** and nanomatrix material **220** may be simply understood to be a combination of the constituents of coating layers **16** that may also include one or more constituents of dispersed particles **214**, depending on the extent of interdiffusion, if any, that occurs between the dispersed particles **214** and the nanomatrix **216**. Similarly, the chemical composition of dispersed particles **214** and particle core material **218** may be simply understood to be a combination of the constituents of particle core **14** that may also include one or more constituents of nanomatrix **216** and nanomatrix material **220**, depending on the extent of interdiffusion, if any, that occurs between the dispersed particles **214** and the nanomatrix **216**.

In an exemplary embodiment, the nanomatrix material **220** has a chemical composition and the particle core material **218** has a chemical composition that is different from that of nanomatrix material **220**, and the differences in the chemical compositions may be configured to provide a selectable and controllable dissolution rate, including a selectable transition from a very low dissolution rate to a very rapid dissolution rate, in response to a controlled change in a property or condition of the wellbore proximate the compact **200**, including a property change in a wellbore fluid that is in contact with the powder compact **200**, as described herein. Nanomatrix **216** may be formed from powder particles **12** having single layer and multilayer coating layers **16**. This design flexibility provides a large number of material combinations, particularly in the case of multilayer coating layers **16**, that can be utilized to tailor the cellular nanomatrix **216** and composition of nanomatrix material **220** by controlling the interaction of the coating layer constituents, both within a given layer, as well as between a coating layer **16** and the particle core **14** with which it is associated or a coating layer **16** of an adjacent powder particle **12**. Several exemplary embodiments that demonstrate this flexibility are provided below.

As illustrated in FIG. 10, in an exemplary embodiment, powder compact **200** is formed from powder particles **12** where the coating layer **16** comprises a single layer, and the resulting nanomatrix **216** between adjacent ones of the plurality of dispersed particles **214** comprises the single metallic coating layer **16** of one powder particle **12**, a bond layer **219** and the single coating layer **16** of another one of the adjacent powder particles **12**. The thickness (t) of bond layer **219** is determined by the extent of the interdiffusion between the single metallic coating layers **16**, and may encompass the entire thickness of nanomatrix **216** or only a portion thereof. In one exemplary embodiment of powder compact **200** formed using a single layer powder **10**, powder compact **200** may include dispersed particles **214** comprising

ing Mg, Al, Zn or Mn, or a combination thereof, as described herein, and nanomatrix 216 may include Al, Zn, Mn, Mg, Mo, W, Cu, Fe, Si, Ca, Co, Ta, Re or Ni, or an oxide, carbide or nitride thereof, or a combination of any of the aforementioned materials, including combinations where the nanomatrix material 220 of cellular nanomatrix 216, including bond layer 219, has a chemical composition and the core material 218 of dispersed particles 214 has a chemical composition that is different than the chemical composition of nanomatrix material 216. The difference in the chemical composition of the nanomatrix material 220 and the core material 218 may be used to provide selectable and controllable dissolution in response to a change in a property of a wellbore, including a wellbore fluid, as described herein. In a further exemplary embodiment of a powder compact 200 formed from a powder 10 having a single coating layer configuration, dispersed particles 214 include Mg, Al, Zn or Mn, or a combination thereof, and the cellular nanomatrix 216 includes Al or Ni, or a combination thereof.

As illustrated in FIG. 15, in another exemplary embodiment, powder compact 200 is formed from powder particles 12 where the coating layer 16 comprises a multilayer coating layer 16 having a plurality of coating layers, and the resulting nanomatrix 216 between adjacent ones of the plurality of dispersed particles 214 comprises the plurality of layers (t) comprising the coating layer 16 of one particle 12, a bond layer 219, and the plurality of layers comprising the coating layer 16 of another one of powder particles 12. In FIG. 15, this is illustrated with a two-layer metallic coating layer 16, but it will be understood that the plurality of layers of multi-layer metallic coating layer 16 may include any desired number of layers. The thickness (t) of the bond layer 219 is again determined by the extent of the interdiffusion between the plurality of layers of the respective coating layers 16, and may encompass the entire thickness of nanomatrix 216 or only a portion thereof. In this embodiment, the plurality of layers comprising each coating layer 16 may be used to control interdiffusion and formation of bond layer 219 and thickness (t).

In one exemplary embodiment of a powder compact 200 made using powder particles 12 with multilayer coating layers 16, the compact includes dispersed particles 214 comprising Mg, Al, Zn or Mn, or a combination thereof, as described herein, and nanomatrix 216 comprises a cellular network of sintered two-layer coating layers 16, as shown in FIG. 3, comprising first layers 22 that are disposed on the dispersed particles 214 and a second layers 24 that are disposed on the first layers 22. First layers 22 include Al or Ni, or a combination thereof, and second layers 24 include Al, Zn, Mn, Mg, Mo, W, Cu, Fe, Si, Ca, Co, Ta, Re or Ni, or a combination thereof. In these configurations, materials of dispersed particles 214 and multilayer coating layer 16 used to form nanomatrix 216 are selected so that the chemical compositions of adjacent materials are different (e.g. dispersed particle/first layer and first layer/second layer).

In another exemplary embodiment of a powder compact 200 made using powder particles 12 with multilayer coating layers 16, the compact includes dispersed particles 214 comprising Mg, Al, Zn or Mn, or a combination thereof, as described herein, and nanomatrix 216 comprises a cellular network of sintered three-layer metallic coating layers 16, as shown in FIG. 4, comprising first layers 22 that are disposed on the dispersed particles 214, second layers 24 that are disposed on the first layers 22 and third layers 26 that are disposed on the second layers 24. First layers 22 include Al or Ni, or a combination thereof; second layers 24 include Al,

Zn, Mn, Mg, Mo, W, Cu, Fe, Si, Ca, Co, Ta, Re or Ni, or an oxide, nitride or carbide thereof, or a combination of any of the aforementioned second layer materials; and the third layers include Al, Zn, Mn, Mg, Mo, W, Cu, Fe, Si, Ca, Co, Ta, Re or Ni, or a combination thereof. The selection of materials is analogous to the selection considerations described herein for powder compact **200** made using two-layer coating layer powders, but must also be extended to include the material used for the third coating layer.

- 10 In yet another exemplary embodiment of a powder compact **200** made using powder particles **12** with multilayer coating layers **16**, the compact includes dispersed particles **214** comprising Mg, Al, Zn or Mn, or a combination thereof, as described herein, and nanomatrix **216** comprise a cellular
  - 15 network of sintered four-layer coating layers **16** comprising first layers **22** that are disposed on the dispersed particles **214**; second layers **24** that are disposed on the first layers **22**; third layers **26** that are disposed on the second layers **24** and fourth layers **28** that are disposed on the third layers **26**. First
  - 20 layers **22** include Al or Ni, or a combination thereof; second layers **24** include Al, Zn, Mn, Mg, Mo, W, Cu, Fe, Si, Ca, Co, Ta, Re or Ni, or an oxide, nitride or carbide thereof, or a combination of any of the aforementioned second layer materials; third layers include Al, Zn, Mn, Mg, Mo, W, Cu,
  - 25 Fe, Si, Ca, Co, Ta, Re or Ni, or an oxide, nitride or carbide thereof, or a combination of any of the aforementioned third layer materials; and fourth layers include Al, Mn, Fe, Co or Ni, or a combination thereof. The selection of materials is analogous to the selection considerations described herein
  - 30 for powder compacts **200** made using two-layer coating layer powders, but must also be extended to include the material used for the third and fourth coating layers

material used for the third and fourth coating layers.

In another exemplary embodiment of a powder compact 200, dispersed particles 214 comprise a metal having a standard oxidation potential less than Zn or a non-metallic material, or a combination thereof, as described herein, and nanomatrix 216 comprises a cellular network of sintered metallic coating layers 16. Suitable non-metallic materials include various ceramics, glasses or forms of carbon, or a combination thereof. Further, in powder compacts 200 that include dispersed particles 214 comprising these metals or non-metallic materials, nanomatrix 216 may include Al, Zn, Mn, Mg, Mo, W, Cu, Fe, Si, Ca, Co, Ta, Re or Ni, or an oxide, carbide or nitride thereof, or a combination of any of the aforementioned materials as nanomatrix material 220.

Referring to FIG. 16, sintered powder compact 200 may comprise a sintered precursor powder compact 100 that includes a plurality of deformed, mechanically bonded powder particles as described herein. Precursor powder compact 100 may be formed by compaction of powder 10 to the point that powder particles 12 are pressed into one another, thereby deforming them and forming interparticle mechanical or other bonds 110 associated with this deformation sufficient to cause the deformed powder particles 12 to 50 adhere to one another and form a green-state powder compact having a green density that is less than the theoretical density of a fully-dense compact of powder 10, due in part to interparticle spaces 15. Compaction may be performed, for example, by isostatically pressing powder 10 at room 55 temperature to provide the deformation and interparticle bonding of powder particles 12 necessary to form precursor powder compact 100.

Sintered and forged powder compacts 200 that include dispersed particles 214 comprising Mg and nanomatrix 216 comprising various nanomatrix materials as described herein have demonstrated an excellent combination of mechanical strength and low density that exemplify the

lightweight, high-strength materials disclosed herein. Examples of powder compacts **200** that have pure Mg dispersed particles **214** and various nanomaterials **216** formed from powders **10** having pure Mg particle cores **14** and various single and multilayer metallic coating layers **16** that include Al, Ni, W or  $\text{Al}_2\text{O}_3$ , or a combination thereof, and that have been made using the method **400** disclosed herein, are listed in a table as FIG. 18. These powders compacts **200** have been subjected to various mechanical and other testing, including density testing, and their dissolution and mechanical property degradation behavior has also been characterized as disclosed herein. The results indicate that these materials may be configured to provide a wide range of selectable and controllable corrosion or dissolution behavior from very low corrosion rates to extremely high corrosion rates, particularly corrosion rates that are both lower and higher than those of powder compacts that do not incorporate the cellular nanomatrix, such as a compact formed from pure Mg powder through the same compaction and sintering processes in comparison to those that include pure Mg dispersed particles in the various cellular nanomaterials described herein. These powder compacts **200** may also be configured to provide substantially enhanced properties as compared to powder compacts formed from pure Mg particles that do not include the nanoscale coatings described herein. For example, referring to FIGS. 18 and 19, powder compacts **200** that include dispersed particles **214** comprising Mg and nanomatrix **216** comprising various nanomaterials **220** described herein have demonstrated room temperature compressive strengths of at least about 37 ksi, and have further demonstrated room temperature compressive strengths in excess of about 50 ksi, both dry and immersed in a solution of 3% KCl at 200° F. In contrast, powder compacts formed from pure Mg powders have a compressive strength of about 20 ksi or less. Strength of the nanomatrix powder metal compact **200** can be further improved by optimizing powder **10**, particularly the weight percentage of the nanoscale metallic coating layers **16** that are used to form cellular nanomatrix **216**. For example, FIG. 25 shows the effect of varying the weight percentage (wt. %), i.e., thickness, of an alumina coating on the room temperature compressive strength of a powder compact **200** of a cellular nanomatrix **216** formed from coated powder particles **12** that include a multilayer ( $\text{Al}/\text{Al}_2\text{O}_3/\text{Al}$ ) metallic coating layer **16** on pure Mg particle cores **14**. In this example, optimal strength is achieved at 4 wt % of alumina, which represents an increase of 21% as compared to that of 0 wt % alumina.

Powder compacts **200** comprising dispersed particles **214** that include Mg and nanomatrix **216** that includes various nanomaterials as described herein have also demonstrated a room temperature shear strength of at least about 20 ksi. This is in contrast with powder compacts formed from pure Mg powders which have room temperature shear strengths of about 8 ksi.

Powder compacts **200** of the types disclosed herein are able to achieve an actual density that is substantially equal to the predetermined theoretical density of a compact material based on the composition of powder **10**, including relative amounts of constituents of particle cores **14** and metallic coating layer **16**, and are also described herein as being fully-dense powder compacts. Powder compacts **200** comprising dispersed particles that include Mg and nanomatrix **216** that includes various nanomaterials as described herein have demonstrated actual densities of about 1.738 g/cm<sup>3</sup> to about 2.50 g/cm<sup>3</sup>, which are substantially

equal to the predetermined theoretical densities, differing by at most 4% from the predetermined theoretical densities.

Powder compacts **200** as disclosed herein may be configured to be selectively and controllably dissolvable in a wellbore fluid in response to a changed condition in a wellbore. Examples of the changed condition that may be exploited to provide selectable and controllable dissolvability include a change in temperature, change in pressure, change in flow rate, change in pH or change in chemical composition of the wellbore fluid, or a combination thereof. An example of a changed condition comprising a change in temperature includes a change in well bore fluid temperature. For example, referring to FIGS. 18 and 20, powder compacts **200** comprising dispersed particles **214** that include Mg and cellular nanomatrix **216** that includes various nanomaterials as described herein have relatively low rates of corrosion in a 3% KCl solution at room temperature that ranges from about 0 to about 11 mg/cm<sup>2</sup>/hr as compared to relatively high rates of corrosion at 200° F. that range from about 1 to about 246 mg/cm<sup>2</sup>/hr depending on different nanoscale coating layers **16**. An example of a changed condition comprising a change in chemical composition includes a change in a chloride ion concentration or pH value, or both, of the wellbore fluid. For example, referring to FIGS. 18 and 21, powder compacts **200** comprising dispersed particles **214** that include Mg and nanomatrix **216** that includes various nanoscale coatings described herein demonstrate corrosion rates in 15% HCl that range from about 4750 mg/cm<sup>2</sup>/hr to about 7432 mg/cm<sup>2</sup>/hr. Thus, selectable and controllable dissolvability in response to a changed condition in the wellbore, namely the change in the wellbore fluid chemical composition from KCl to HCl, may be used to achieve a characteristic response as illustrated graphically in FIG. 22, which illustrates that at a selected predetermined critical service time (CST) a changed condition may be imposed upon powder compact **200** as it is applied in a given application, such as a wellbore environment, that causes a controllable change in a property of powder compact **200** in response to a changed condition in the environment in which it is applied. For example, at a predetermined CST changing a wellbore fluid that is in contact with powder contact **200** from a first fluid (e.g. KCl) that provides a first corrosion rate and an associated weight loss or strength as a function of time to a second wellbore fluid (e.g., HCl) that provides a second corrosion rate and associated weight loss and strength as a function of time, wherein the corrosion rate associated with the first fluid is much less than the corrosion rate associated with the second fluid. This characteristic response to a change in wellbore fluid conditions may be used, for example, to associate the critical service time with a dimension loss limit or a minimum strength needed for a particular application, such that when a wellbore tool or component formed from powder compact **200** as disclosed herein is no longer needed in service in the wellbore (e.g., the CST) the condition in the wellbore (e.g., the chloride ion concentration of the wellbore fluid) may be changed to cause the rapid dissolution of powder compact **200** and its removal from the wellbore. In the example described above, powder compact **200** is selectively dissolvable at a rate that ranges from about 0 to about 7000 mg/cm<sup>2</sup>/hr. This range of response provides, for example the ability to remove a 3 inch diameter ball formed from this material from a wellbore by altering the wellbore fluid in less than one hour. The selectable and controllable dissolvability behavior described above, coupled with the excellent strength and low density properties described herein, define a new engineered dispersed particle-nanoma-

trix material that is configured for contact with a fluid and configured to provide a selectable and controllable transition from one of a first strength condition to a second strength condition that is lower than a functional strength threshold, or a first weight loss amount to a second weight loss amount that is greater than a weight loss limit, as a function of time in contact with the fluid. The dispersed particle-nanomatrix composite is characteristic of the powder compacts 200 described herein and includes a cellular nanomatrix 216 of nanomatrix material 220, a plurality of dispersed particles 214 including particle core material 218 that is dispersed within the matrix. Nanomatrix 216 is characterized by a solid-state bond layer 219 which extends throughout the nanomatrix. The time in contact with the fluid described above may include the CST as described above. The CST may include a predetermined time that is desired or required to dissolve a predetermined portion of the powder compact 200 that is in contact with the fluid. The CST may also include a time corresponding to a change in the property of the engineered material or the fluid, or a combination thereof. In the case of a change of property of the engineered material, the change may include a change of a temperature of the engineered material. In the case where there is a change in the property of the fluid, the change may include the change in a fluid temperature, pressure, flow rate, chemical composition or pH or a combination thereof. Both the engineered material and the change in the property of the engineered material or the fluid, or a combination thereof, may be tailored to provide the desired CST response characteristic, including the rate of change of the particular property (e.g., weight loss, loss of strength) both prior to the CST (e.g., Stage 1) and after the CST (e.g., Stage 2), as illustrated in FIG. 22.

Referring to FIG. 17, a method 400 of making a powder compact 200. Method 400 includes forming 410 a coated metallic powder 10 comprising powder particles 12 having particle cores 14 with nanoscale metallic coating layers 16 disposed thereon, wherein the metallic coating layers 16 have a chemical composition and the particle cores 14 have a chemical composition that is different than the chemical composition of the metallic coating material 16. Method 400 also includes forming 420 a powder compact by applying a predetermined temperature and a predetermined pressure to the coated powder particles sufficient to sinter them by solid-phase sintering of the coated layers of the plurality of the coated particle powders 12 to form a substantially-continuous, cellular nanomatrix 216 of a nanomatrix material 220 and a plurality of dispersed particles 214 dispersed within nanomatrix 216 as described herein.

Forming 410 of coated metallic powder 10 comprising powder particles 12 having particle cores 14 with nanoscale metallic coating layers 16 disposed thereon may be performed by any suitable method. In an exemplary embodiment, forming 410 includes applying the metallic coating layers 16, as described herein, to the particle cores 14, as described herein, using fluidized bed chemical vapor deposition (FBCVD) as described herein. Applying the metallic coating layers 16 may include applying single-layer metallic coating layers 16 or multilayer metallic coating layers 16 as described herein. Applying the metallic coating layers 16 may also include controlling the thickness of the individual layers as they are being applied, as well as controlling the overall thickness of metallic coating layers 16. Particle cores 14 may be formed as described herein.

Forming 420 of the powder compact 200 may include any suitable method of forming a fully-dense compact of powder 10. In an exemplary embodiment, forming 420 includes

dynamic forging of a green-density precursor powder compact 100 to apply a predetermined temperature and a predetermined pressure sufficient to sinter and deform the powder particles and form a fully-dense nanomatrix 216 and dispersed particles 214 as described herein. Dynamic forging as used herein means dynamic application of a load at temperature and for a time sufficient to promote sintering of the metallic coating layers 16 of adjacent powder particles 12, and may preferably include application of a dynamic forging load at a predetermined loading rate for a time and at a temperature sufficient to form a sintered and fully-dense powder compact 200. In an exemplary embodiment, dynamic forging included: 1) heating a precursor or green-state powder compact 100 to a predetermined solid phase sintering temperature, such as, for example, a temperature sufficient to promote interdiffusion between metallic coating layers 16 of adjacent powder particles 12; 2) holding the precursor powder compact 100 at the sintering temperature for a predetermined hold time, such as, for example, a time sufficient to ensure substantial uniformity of the sintering temperature throughout the precursor compact 100; 3) forging the precursor powder compact 100 to full density, such as, for example, by applying a predetermined forging pressure according to a predetermined pressure schedule or ramp rate sufficient to rapidly achieve full density while holding the compact at the predetermined sintering temperature; and 4) cooling the compact to room temperature. The predetermined pressure and predetermined temperature applied during forming 420 will include a sintering temperature,  $T_s$ , and forging pressure,  $P_F$ , as described herein that will ensure solid-state sintering and deformation of the powder particles 12 to form fully-dense powder compact 200, including solid-state bond 217 and bond layer 219. The steps of heating to and holding the precursor powder compact 100 at the predetermined sintering temperature for the predetermined time may include any suitable combination of temperature and time, and will depend, for example, on the powder 10 selected, including the materials used for particle core 14 and metallic coating layer 16, the size of the precursor powder compact 100, the heating method used and other factors that influence the time needed to achieve the desired temperature and temperature uniformity within precursor powder compact 100. In the step of forging, the predetermined pressure may include any suitable pressure and pressure application schedule or pressure ramp rate sufficient to achieve a fully-dense powder compact 200, and will depend, for example, on the material properties of the powder particles 12 selected, including temperature dependent stress/strain characteristics (e.g., stress/strain rate characteristics), interdiffusion and metallurgical thermodynamic and phase equilibria characteristics, dislocation dynamics and other material properties. For example, the maximum forging pressure of dynamic forging and the forging schedule (i.e., the pressure ramp rates that correspond to strain rates employed) may be used to tailor the mechanical strength and toughness of the powder compact. The maximum forging pressure and forging ramp rate (i.e., strain rate) is the pressure just below the compact cracking pressure, i.e., where dynamic recovery processes are unable to relieve strain energy in the compact microstructure without the formation of a crack in the compact. For example, for applications that require a powder compact that has relatively higher strength and lower toughness, relatively higher forging pressures and ramp rates may be used. If relatively higher toughness of the powder compact is needed, relatively lower forging pressures and ramp rates may be used.

For certain exemplary embodiments of powders 10 described herein and precursor compacts 100 of a size sufficient to form many wellbore tools and components, predetermined hold times of about 1 to about 5 hours may be used. The predetermined sintering temperature,  $T_s$ , will preferably be selected as described herein to avoid melting of either particle cores 14 and metallic coating layers 16 as they are transformed during method 400 to provide dispersed particles 214 and nanomatrix 216. For these embodiments, dynamic forging may include application of a forging pressure, such as by dynamic pressing to a maximum of about 80 ksi at pressure ramp rate of about 0.5 to about 2 ksi/second.

In an exemplary embodiment where particle cores 14 included Mg and metallic coating layer 16 included various single and multilayer coating layers as described herein, such as various single and multilayer coatings comprising Al, the dynamic forging was performed by sintering at a temperature,  $T_s$ , of about 450° C. to about 470° C. for up to about 1 hour without the application of a forging pressure, followed by dynamic forging by application of isostatic pressures at ramp rates between about 0.5 to about 2 ksi/second to a maximum pressure,  $P_s$ , of about 30 ksi to about 60 ksi, which resulted in forging cycles of 15 seconds to about 120 seconds. The short duration of the forging cycle is a significant advantage as it limits interdiffusion, including interdiffusion within a given metallic coating layer 16, interdiffusion between adjacent metallic coating layers 16 and interdiffusion between metallic coating layers 16 and particle cores 14, to that needed to form metallurgical bond 217 and bond layer 219, while also maintaining the desirable equiaxed dispersed particle 214 shape with the integrity of cellular nanomatrix 216 strengthening phase. The duration of the dynamic forging cycle is much shorter than the forming cycles and sintering times required for conventional powder compact forming processes, such as hot isostatic pressing (HIP), pressure assisted sintering or diffusion sintering.

Method 400 may also optionally include forming 430 a precursor powder compact by compacting the plurality of coated powder particles 12 sufficiently to deform the particles and form interparticle bonds to one another and form the precursor powder compact 100 prior to forming 420 the powder compact. Compacting may include pressing, such as isostatic pressing, of the plurality of powder particles 12 at room temperature to form precursor powder compact 100. Compacting 430 may be performed at room temperature. In an exemplary embodiment, powder 10 may include particle cores 14 comprising Mg and forming 430 the precursor powder compact may be performed at room temperature at an isostatic pressure of about 10 ksi to about 60 ksi.

Method 400 may optionally also include intermixing 440 a second powder 30 into powder 10 as described herein prior to the forming 420 the powder compact, or forming 430 the precursor powder compact.

Without being limited by theory, powder compacts 200 are formed from coated powder particles 12 that include a particle core 14 and associated core material 18 as well as a metallic coating layer 16 and an associated metallic coating material 20 to form a substantially-continuous, three-dimensional, cellular nanomatrix 216 that includes a nanomatrix material 220 formed by sintering and the associated diffusion bonding of the respective coating layers 16 that includes a plurality of dispersed particles 214 of the particle core materials 218. This unique structure may include metastable combinations of materials that would be very difficult or impossible to form by solidification from a melt having

the same relative amounts of the constituent materials. The coating layers and associated coating materials may be selected to provide selectable and controllable dissolution in a predetermined fluid environment, such as a wellbore environment, where the predetermined fluid may be a commonly used wellbore fluid that is either injected into the wellbore or extracted from the wellbore. As will be further understood from the description herein, controlled dissolution of the nanomatrix exposes the dispersed particles of the core materials. The particle core materials may also be selected to also provide selectable and controllable dissolution in the wellbore fluid. Alternately, they may also be selected to provide a particular mechanical property, such as compressive strength or sheer strength, to the powder compact 200, without necessarily providing selectable and controlled dissolution of the core materials themselves, since selectable and controlled dissolution of the nanomatrix material surrounding these particles will necessarily release them so that they are carried away by the wellbore fluid. The microstructural morphology of the substantially-continuous, cellular nanomatrix 216, which may be selected to provide a strengthening phase material, with dispersed particles 214, which may be selected to provide equiaxed dispersed particles 214, provides these powder compacts with enhanced mechanical properties, including compressive strength and sheer strength, since the resulting morphology of the nanomatrix/dispersed particles can be manipulated to provide strengthening through the processes that are akin to traditional strengthening mechanisms, such as grain size reduction, solution hardening through the use of impurity atoms, precipitation or age hardening and strength/work hardening mechanisms. The nanomatrix/dispersed particle structure tends to limit dislocation movement by virtue of the numerous particle nanomatrix interfaces, as well as interfaces between discrete layers within the nanomatrix material as described herein. This is exemplified in the fracture behavior of these materials, as illustrated in FIGS. 23 and 24. In FIG. 23, a powder compact 200 made using uncoated pure Mg powder and subjected to a shear stress sufficient to induce failure demonstrated intergranular fracture. In contrast, in FIG. 24, a powder compact 200 made using powder particles 12 having pure Mg powder particle cores 14 to form dispersed particles 214 and metallic coating layers 16 that includes Al to form nanomatrix 216 and subjected to a shear stress sufficient to induce failure demonstrated transgranular fracture and a substantially higher fracture stress as described herein. Because these materials have high-strength characteristics, the core material and coating material may be selected to utilize low density materials or other low density materials, such as low-density metals, ceramics, glasses or carbon, that otherwise would not provide the necessary strength characteristics for use in the desired applications, including wellbore tools and components.

While one or more embodiments have been shown and described, modifications and substitutions may be made thereto without departing from the spirit and scope of the invention. Accordingly, it is to be understood that the present invention has been described by way of illustrations and not limitation.

The invention claimed is:

1. A metallic powder comprising a plurality of metallic powder particles disposed in a powder compact, each powder particle comprising:
  - a particle core, the particle core comprises a core material comprising Mg, Al, Zn or Mn, or a combination thereof; and

## 25

a metallic coating layer disposed on the particle core and comprising a metallic coating material, wherein the metallic coating layer comprises a plurality of coating layers, and wherein a first coating layer comprises Al, a second coating layer comprises Al, Zn, Mn, Mg, Mo, W, Cu, Fe, Si, Ca, Co, Ta, Re, or Ni, or an oxide, nitride or carbide thereof, or a combination of any of the aforementioned second coating layer materials, and a third coating layer comprises Al, Zn, Mn, Mg, Mo, W, Fe, Si, Ca, Co, Ta, Re, or Ni, or a combination thereof, 10 wherein the first coating layer has a chemical composition that is different than a chemical composition of the second coating layer, and the chemical composition of the second coating layer is different than a chemical composition of the third layer, and wherein the powder compact of the powder particles is selectively and controllably dissolvable in a predetermined wellbore fluid comprising potassium chloride, hydrochloric acid, calcium chloride, calcium bromide, or zinc bromide.

2. The metal powder of claim 1, wherein the particle core 20 has a diameter of about 5  $\mu\text{m}$  to about 300  $\mu\text{m}$ .

3. The metal powder of claim 1, wherein the core material is a binary Mg—Zn, Al—Zn, Mg—Mn, Zn—Mn alloy, or a 25 tertiary Mg—Zn—Y alloy.

4. The metal powder of claim 1, wherein the core material is a tertiary Mg—Al—X alloy, wherein X is Zn, Mn, Si, Ca or Y, or a combination thereof.

5. The metal powder of claim 4, wherein the Mg—Al—X 30 alloy comprises, by weight, up to about 85% Mg, up to about 15% Al and up to about 5% X.

6. The metal powder of claim 1, wherein the core material further comprises a rare earth element.

7. The metal powder of claim 6, wherein the rare earth element comprises, by weight, less than about 5% of the 35 particle core.

8. The metal powder of claim 1, wherein the metallic coating material has a chemical composition and the core material has a chemical composition that is different than the chemical composition of the coating material.

9. The metal powder of claim 1, wherein the coating layer 40 has a thickness of about 25 nm to about 2500 nm.

10. The metal powder of claim 1, further comprising a fourth coating layer that is disposed on the third coating layer.

11. The metal powder of claim 1, wherein the fourth 45 coating layer comprises Al, Mn, Fe, Co or Ni, or a combination thereof, and wherein the chemical composition of the third coating layer is different than a chemical composition of the fourth coating layer.

12. A metallic powder comprising a plurality of metallic 50 powder particles, each powder particle comprising: a particle core, the particle core comprises a core material comprising a metal having a standard oxidation potential less than Zn, ceramic, glass, or carbon, or a combination thereof; and a metallic coating layer disposed on the particle core and comprising a metallic coating material, wherein the metallic coating layer comprises a plurality of coating 55

## 26

layers, and wherein a first coating layer comprises Al, a second coating layer comprises Al, Zn, Mn, Mg, Mo, W, Cu, Fe, Si, Ca, Co, Ta, Re, or Ni, or an oxide, nitride or carbide thereof, or a combination of any of the aforementioned second coating layer materials, and a third coating layer comprises Al, Zn, Mn, Mg, Mo, W, Fe, Si, Ca, Co, Ta, Re, or Ni, or a combination thereof, wherein the first coating layer has a chemical composition that is different than a chemical composition of the second coating layer, and the chemical composition of the second coating layer is different than a chemical composition of the third layer, and wherein the second coating layer is configured to provide at least one of enhanced interlayer adhesion, enhanced strength of the overall metallic coating layer, or limited interlayer diffusion.

13. The metallic powder of claim 12, wherein the metallic coating material has a chemical composition and the core material has a chemical composition that is different than the chemical composition of the coating material.

14. A method of making a metal powder, comprising: forming a metal powder comprising a plurality of powder particles of a binary Mg—Zn, Mg—Mn, Al—Zn, Al—Mn, or Zn—Mn alloy, or a tertiary Mg—Zn—Y alloy, or a tertiary Mg—Al—X alloy, wherein X is Zn, Mn, Si, Ca, or Y, or a combination thereof, as a core material for use as a plurality of particle cores; and depositing a metallic coating layer on each of the plurality of particle cores, wherein the metallic coating layer comprises a plurality of coating layers, and wherein a first coating layer comprises Al, a second coating layer comprises Al, Zn, Mn, Mg, Mo, W, Cu, Fe, Si, Ca, Co, Ta, Re, or Ni, or an oxide, nitride or carbide thereof, or a combination of any of the aforementioned second coating layer materials, and a third coating layer comprises Al, Zn, Mn, Mg, Mo, W, Fe, Si, Ca, Co, Ta, Re, or Ni, or a combination thereof, wherein the first coating layer has a chemical composition that is different than a chemical composition of the second coating layer, and the chemical composition of the second coating layer is different than a chemical composition of the third layer, and wherein the second coating layer is configured to provide at least one of enhanced interlayer adhesion, enhanced strength of the overall metallic coating layer, or limited interlayer diffusion.

15. The method of claim 14, wherein forming the metal powder comprises vacuum spray forming or inert gas spray forming.

16. The method of claim 14, wherein depositing the coating layer comprises depositing the coating material by fluidized bed chemical vapor deposition.

17. The method of claim 14, wherein depositing the metallic coating layer comprises depositing the first coating layer comprising Al or Ni, or a combination thereof, on the particle core.

\* \* \* \* \*